



US009347119B2

(12) **United States Patent**  
**Xu**

(10) **Patent No.:** **US 9,347,119 B2**  
(45) **Date of Patent:** **May 24, 2016**

(54) **DEGRADABLE HIGH SHOCK IMPEDANCE MATERIAL**

(75) Inventor: **Zhiyue Xu**, Cypress, TX (US)

(73) Assignee: **BAKER HUGHES INCORPORATED**, Houston, TX (US)

(\*) Notice: Subject to any disclaimer, the term of this patent is extended or adjusted under 35 U.S.C. 154(b) by 1106 days.

(21) Appl. No.: **13/225,413**

(22) Filed: **Sep. 3, 2011**

(65) **Prior Publication Data**

US 2013/0055852 A1 Mar. 7, 2013

(51) **Int. Cl.**

*C22C 29/00* (2006.01)  
*C22C 32/00* (2006.01)  
*B22F 1/00* (2006.01)  
*B22F 1/02* (2006.01)  
*B22F 3/04* (2006.01)  
*B22F 3/17* (2006.01)  
*B22F 3/18* (2006.01)  
*B22F 3/20* (2006.01)

(52) **U.S. Cl.**

CPC ..... *C22C 29/00* (2013.01); *C22C 32/00* (2013.01); *B22F 1/0044* (2013.01); *B22F 1/025* (2013.01); *B22F 3/04* (2013.01); *B22F 3/17* (2013.01); *B22F 3/18* (2013.01); *B22F 3/20* (2013.01); *Y10T 428/249921* (2015.04); *Y10T 428/268* (2015.01)

(58) **Field of Classification Search**

USPC ..... 75/228, 230  
See application file for complete search history.

(56) **References Cited**

U.S. PATENT DOCUMENTS

1,468,905 A 9/1923 Herman  
2,238,895 A 4/1941 Gage

2,261,292 A 11/1941 Salnikov  
2,294,648 A 9/1942 Ansel et al.  
2,301,624 A 11/1942 Holt  
2,394,843 A 2/1946 Cooke et al.  
2,754,910 A 7/1956 Derrick et al.  
2,983,634 A 5/1961 Budininkas et al.  
3,057,405 A 10/1962 Mallinger

(Continued)

FOREIGN PATENT DOCUMENTS

CA 2783241 A1 6/2011  
CA 2783346 A1 6/2011  
CN 1255879 A 6/2000

(Continued)

OTHER PUBLICATIONS

W. Walters, P. Peregino, R. Summers, and D. Leidel; "A Study of Jets from Unsintered-Powder Metal Lined Nonprecision Small-Caliber Shaped Charges", Army Research Laboratory, Aberdeen Proving Ground, MD 21005-5066; Feb. 2001.

(Continued)

*Primary Examiner* — Jessee Roe

*Assistant Examiner* — Ngoclan T Mai

(74) *Attorney, Agent, or Firm* — Cantor Colburn LLP

(57) **ABSTRACT**

A selectively corrodible powder compact that may be used to make the components of a selectively corrodible perforating system is disclosed. The selectively corrodible powder compact includes a cellular nanomatrix comprising a nanomatrix material. The selectively corrodible powder compact also includes a plurality of dispersed particles comprising a particle core material having a density of about  $7.5 \text{ g/cm}^3$  or more, dispersed in the cellular nanomatrix. The selectively corrodible powder compact further includes a bond layer extending throughout the cellular nanomatrix between the dispersed particles.

**25 Claims, 5 Drawing Sheets**



| (56)                  | References Cited |                      |             |         |                       |  |
|-----------------------|------------------|----------------------|-------------|---------|-----------------------|--|
| U.S. PATENT DOCUMENTS |                  |                      |             |         |                       |  |
| 3,106,959 A           | 10/1963          | Huitt et al.         | 4,889,187 A | 12/1989 | Terrell et al.        |  |
| 3,152,009 A           | 10/1964          | Delong               | 4,890,675 A | 1/1990  | Dew                   |  |
| 3,196,949 A           | 7/1965           | Thomas               | 4,909,320 A | 3/1990  | Hebert et al.         |  |
| 3,242,988 A           | 3/1966           | McGuire et al.       | 4,929,415 A | 5/1990  | Okazaki               |  |
| 3,316,748 A           | 5/1967           | Lang et al.          | 4,932,474 A | 6/1990  | Schroeder, Jr. et al. |  |
| 3,326,291 A           | 6/1967           | Zandmer et al.       | 4,938,309 A | 7/1990  | Endy                  |  |
| 3,343,537 A           | 9/1967           | Zandmer              | 4,938,809 A | 7/1990  | Das et al.            |  |
| 3,347,317 A           | 10/1967          | Zandemer             | 4,944,351 A | 7/1990  | Eriksen et al.        |  |
| 3,347,714 A           | 10/1967          | Broverman et al.     | 4,949,788 A | 8/1990  | Szarka et al.         |  |
| 3,390,724 A           | 7/1968           | Caldwell             | 4,952,902 A | 8/1990  | Kawaguchi et al.      |  |
| 3,395,758 A           | 8/1968           | Kelly et al.         | 4,975,412 A | 12/1990 | Okazaki et al.        |  |
| 3,406,101 A           | 10/1968          | Kilpatrick           | 4,977,958 A | 12/1990 | Miller                |  |
| 3,465,181 A           | 9/1969           | Colby et al.         | 4,981,177 A | 1/1991  | Carmody et al.        |  |
| 3,513,230 A           | 5/1970           | Rhees et al.         | 4,986,361 A | 1/1991  | Mueller et al.        |  |
| 3,637,446 A           | 1/1972           | Elliott et al.       | 4,997,622 A | 3/1991  | Regazzoni et al.      |  |
| 3,645,331 A           | 2/1972           | Maurer et al.        | 5,006,044 A | 4/1991  | Walker, Sr. et al.    |  |
| 3,765,484 A           | 10/1973          | Hamby, Jr. et al.    | 5,010,955 A | 4/1991  | Springer              |  |
| 3,768,563 A           | 10/1973          | Blount               | 5,036,921 A | 8/1991  | Pittard et al.        |  |
| 3,775,823 A           | 12/1973          | Adolph et al.        | 5,048,611 A | 9/1991  | Cochran               |  |
| 3,878,889 A           | 4/1975           | Seabourn             | 5,049,165 A | 9/1991  | Tselesin              |  |
| 3,894,850 A           | 7/1975           | Kovalchuk et al.     | 5,061,323 A | 10/1991 | DeLucia               |  |
| 3,924,677 A           | 12/1975          | Prenner et al.       | 5,063,775 A | 11/1991 | Walker, Sr. et al.    |  |
| 4,010,583 A           | 3/1977           | Highberg             | 5,073,207 A | 12/1991 | Faure et al.          |  |
| 4,039,717 A           | 8/1977           | Titus                | 5,074,361 A | 12/1991 | Brisco et al.         |  |
| 4,050,529 A           | 9/1977           | Tagirov et al.       | 5,076,869 A | 12/1991 | Bourell et al.        |  |
| 4,157,732 A           | 6/1979           | Fonner               | 5,084,088 A | 1/1992  | Okazaki               |  |
| 4,248,307 A           | 2/1981           | Silberman et al.     | 5,087,304 A | 2/1992  | Chang et al.          |  |
| 4,372,384 A           | 2/1983           | Kinney               | 5,090,480 A | 2/1992  | Pittard et al.        |  |
| 4,373,584 A           | 2/1983           | Silberman et al.     | 5,095,988 A | 3/1992  | Bode                  |  |
| 4,373,952 A           | 2/1983           | Parent               | 5,103,911 A | 4/1992  | Heijnen               |  |
| 4,374,543 A           | 2/1983           | Richardson           | 5,117,915 A | 6/1992  | Mueller et al.        |  |
| 4,384,616 A           | 5/1983           | Dellinger            | 5,161,614 A | 11/1992 | Wu et al.             |  |
| 4,395,440 A           | 7/1983           | Abe et al.           | 5,178,216 A | 1/1993  | Giroux et al.         |  |
| 4,399,871 A           | 8/1983           | Adkins et al.        | 5,181,571 A | 1/1993  | Mueller et al.        |  |
| 4,407,368 A           | 10/1983          | Erbstoesser          | 5,183,631 A | 2/1993  | Kugimiya et al.       |  |
| 4,422,508 A           | 12/1983          | Rutledge, Jr. et al. | 5,188,182 A | 2/1993  | Echols, III et al.    |  |
| 4,452,311 A           | 6/1984           | Speegle et al.       | 5,188,183 A | 2/1993  | Hopmann et al.        |  |
| 4,475,729 A           | 10/1984          | Costigan             | 5,204,055 A | 4/1993  | Sachs et al.          |  |
| 4,498,543 A           | 2/1985           | Pye et al.           | 5,222,867 A | 6/1993  | Walker, Sr. et al.    |  |
| 4,499,048 A           | 2/1985           | Hanejko              | 5,226,483 A | 7/1993  | Williamson, Jr.       |  |
| 4,499,049 A           | 2/1985           | Hanejko              | 5,228,518 A | 7/1993  | Wilson et al.         |  |
| 4,526,840 A           | 7/1985           | Jarabek              | 5,234,055 A | 8/1993  | Cornette              |  |
| 4,534,414 A           | 8/1985           | Pringle              | 5,252,365 A | 10/1993 | White                 |  |
| 4,539,175 A           | 9/1985           | Lichti et al.        | 5,253,714 A | 10/1993 | Davis et al.          |  |
| 4,554,986 A           | 11/1985          | Jones                | 5,271,468 A | 12/1993 | Streich et al.        |  |
| 4,640,354 A           | 2/1987           | Boisson              | 5,282,509 A | 2/1994  | Schurr, III           |  |
| 4,664,962 A           | 5/1987           | DesMarais, Jr.       | 5,292,478 A | 3/1994  | Scorey                |  |
| 4,668,470 A           | 5/1987           | Gilman et al.        | 5,293,940 A | 3/1994  | Hromas et al.         |  |
| 4,673,549 A           | 6/1987           | Ecer                 | 5,304,260 A | 4/1994  | Aikawa et al.         |  |
| 4,674,572 A           | 6/1987           | Gallus               | 5,309,874 A | 5/1994  | Willermet et al.      |  |
| 4,678,037 A           | 7/1987           | Smith                | 5,310,000 A | 5/1994  | Arterbury et al.      |  |
| 4,681,133 A           | 7/1987           | Weston               | 5,316,598 A | 5/1994  | Chang et al.          |  |
| 4,688,641 A           | 8/1987           | Knieriem             | 5,318,746 A | 6/1994  | Lashmore              |  |
| 4,693,863 A           | 9/1987           | Del Corso et al.     | 5,380,473 A | 1/1995  | Bogue et al.          |  |
| 4,703,807 A           | 11/1987          | Weston               | 5,387,380 A | 2/1995  | Cima et al.           |  |
| 4,706,753 A           | 11/1987          | Ohkochi et al.       | 5,392,860 A | 2/1995  | Ross                  |  |
| 4,708,202 A           | 11/1987          | Sukup et al.         | 5,394,941 A | 3/1995  | Venditto et al.       |  |
| 4,708,208 A           | 11/1987          | Halbardier           | 5,398,754 A | 3/1995  | Dinhoble              |  |
| 4,709,761 A           | 12/1987          | Setterberg, Jr.      | 5,407,011 A | 4/1995  | Layout                |  |
| 4,714,116 A           | 12/1987          | Brunner              | 5,409,555 A | 4/1995  | Fujita et al.         |  |
| 4,716,964 A           | 1/1988           | Erbstoesser et al.   | 5,411,082 A | 5/1995  | Kennedy               |  |
| 4,721,159 A           | 1/1988           | Ohkochi et al.       | 5,417,285 A | 5/1995  | Van Buskirk et al.    |  |
| 4,738,599 A           | 4/1988           | Shilling             | 5,425,424 A | 6/1995  | Reinhardt et al.      |  |
| 4,741,973 A           | 5/1988           | Condit et al.        | 5,427,177 A | 6/1995  | Jordan, Jr. et al.    |  |
| 4,768,588 A           | 9/1988           | Kupsa                | 5,435,392 A | 7/1995  | Kennedy               |  |
| 4,775,598 A           | 10/1988          | Jaecel               | 5,439,051 A | 8/1995  | Kennedy et al.        |  |
| 4,784,226 A           | 11/1988          | Wyatt                | 5,454,430 A | 10/1995 | Kennedy et al.        |  |
| 4,805,699 A           | 2/1989           | Halbardier           | 5,456,317 A | 10/1995 | Hood, III et al.      |  |
| 4,817,725 A           | 4/1989           | Jenkins              | 5,456,327 A | 10/1995 | Denton et al.         |  |
| 4,834,184 A           | 5/1989           | Streich et al.       | 5,464,062 A | 11/1995 | Blizzard, Jr.         |  |
| H635 H                | 6/1989           | Johnson et al.       | 5,472,048 A | 12/1995 | Kennedy et al.        |  |
| 4,850,432 A           | 7/1989           | Porter et al.        | 5,474,131 A | 12/1995 | Jordan, Jr. et al.    |  |
| 4,853,056 A           | 8/1989           | Hoffman              | 5,477,923 A | 12/1995 | Jordan, Jr. et al.    |  |
| 4,869,324 A           | 9/1989           | Holder               | 5,479,986 A | 1/1996  | Gano et al.           |  |
| 4,869,325 A           | 9/1989           | Halbardier           | 5,507,439 A | 4/1996  | Story                 |  |
|                       |                  |                      | 5,526,880 A | 6/1996  | Jordan, Jr. et al.    |  |
|                       |                  |                      | 5,526,881 A | 6/1996  | Martin et al.         |  |
|                       |                  |                      | 5,529,746 A | 6/1996  | Knoss et al.          |  |
|                       |                  |                      | 5,533,573 A | 7/1996  | Jordan, Jr. et al.    |  |

| (56)                  | References Cited |                    |              |         |                     |
|-----------------------|------------------|--------------------|--------------|---------|---------------------|
| U.S. PATENT DOCUMENTS |                  |                    |              |         |                     |
| 5,536,485 A           | 7/1996           | Kume et al.        | 6,349,766 B1 | 2/2002  | Bussear et al.      |
| 5,558,153 A           | 9/1996           | Holcombe et al.    | 6,354,379 B2 | 3/2002  | Miszewski et al.    |
| 5,607,017 A           | 3/1997           | Owens et al.       | 6,357,332 B1 | 3/2002  | Vecchio             |
| 5,623,993 A           | 4/1997           | Van Buskirk et al. | 6,371,206 B1 | 4/2002  | Mills               |
| 5,623,994 A           | 4/1997           | Robinson           | 6,372,346 B1 | 4/2002  | Toth                |
| 5,636,691 A           | 6/1997           | Hendrickson et al. | 6,382,244 B2 | 5/2002  | Vann                |
| 5,641,023 A           | 6/1997           | Ross et al.        | 6,390,195 B1 | 5/2002  | Nguyen et al.       |
| 5,647,444 A           | 7/1997           | Williams           | 6,390,200 B1 | 5/2002  | Allamon et al.      |
| 5,665,289 A           | 9/1997           | Chung et al.       | 6,394,185 B1 | 5/2002  | Constien            |
| 5,677,372 A           | 10/1997          | Yamamoto et al.    | 6,397,950 B1 | 6/2002  | Streich et al.      |
| 5,685,372 A           | 11/1997          | Gano               | 6,403,210 B1 | 6/2002  | Stuivinga et al.    |
| 5,701,576 A           | 12/1997          | Fujita et al.      | 6,408,946 B1 | 6/2002  | Marshall et al.     |
| 5,707,214 A           | 1/1998           | Schmidt            | 6,419,023 B1 | 7/2002  | George et al.       |
| 5,709,269 A           | 1/1998           | Head               | 6,439,313 B1 | 8/2002  | Thomeer et al.      |
| 5,720,344 A           | 2/1998           | Newman             | 6,457,525 B1 | 10/2002 | Scott               |
| 5,728,195 A           | 3/1998           | Eastman et al.     | 6,467,546 B2 | 10/2002 | Allamon et al.      |
| 5,765,639 A           | 6/1998           | Muth               | 6,470,965 B1 | 10/2002 | Winzer              |
| 5,772,735 A           | 6/1998           | Sehgal et al.      | 6,491,097 B1 | 12/2002 | Oneal et al.        |
| 5,782,305 A           | 7/1998           | Hicks              | 6,491,116 B2 | 12/2002 | Berscheidt et al.   |
| 5,797,454 A           | 8/1998           | Hipp               | 6,513,598 B2 | 2/2003  | Moore et al.        |
| 5,826,652 A           | 10/1998          | Tapp               | 6,540,033 B1 | 4/2003  | Sullivan et al.     |
| 5,826,661 A           | 10/1998          | Parker et al.      | 6,543,543 B2 | 4/2003  | Muth                |
| 5,829,520 A           | 11/1998          | Johnson            | 6,561,275 B2 | 5/2003  | Glass et al.        |
| 5,836,396 A           | 11/1998          | Norman             | 6,588,507 B2 | 7/2003  | Dusterhoff et al.   |
| 5,857,521 A           | 1/1999           | Ross et al.        | 6,591,915 B2 | 7/2003  | Burris et al.       |
| 5,881,816 A           | 3/1999           | Wright             | 6,601,648 B2 | 8/2003  | Ebinger             |
| 5,896,819 A           | 4/1999           | Turila et al.      | 6,601,650 B2 | 8/2003  | Sundararajan        |
| 5,902,424 A           | 5/1999           | Fujita et al.      | 6,609,569 B2 | 8/2003  | Howlett et al.      |
| 5,934,372 A           | 8/1999           | Muth               | 6,612,826 B1 | 9/2003  | Bauer et al.        |
| 5,941,309 A           | 8/1999           | Appleton           | 6,613,383 B1 | 9/2003  | George et al.       |
| 5,960,881 A           | 10/1999          | Allamon et al.     | 6,699,305 B2 | 3/2004  | Myrick              |
| 5,985,466 A           | 11/1999          | Atarashi et al.    | 6,713,177 B2 | 3/2004  | George et al.       |
| 5,990,051 A           | 11/1999          | Ischy et al.       | 6,715,541 B2 | 4/2004  | Pedersen et al.     |
| 5,992,452 A           | 11/1999          | Nelson, II         | 6,719,051 B2 | 4/2004  | Hailey, Jr. et al.  |
| 5,992,520 A           | 11/1999          | Schultz et al.     | 6,755,249 B2 | 6/2004  | Robison et al.      |
| 6,007,314 A           | 12/1999          | Nelson, II         | 6,776,228 B2 | 8/2004  | Pedersen et al.     |
| 6,024,915 A           | 2/2000           | Kume et al.        | 6,779,599 B2 | 8/2004  | Mullins et al.      |
| 6,032,735 A           | 3/2000           | Echols             | 6,799,638 B2 | 10/2004 | Butterfield, Jr.    |
| 6,036,777 A           | 3/2000           | Sachs              | 6,810,960 B2 | 11/2004 | Pia                 |
| 6,047,773 A           | 4/2000           | Zeltmann et al.    | 6,817,414 B2 | 11/2004 | Lee                 |
| 6,050,340 A           | 4/2000           | Scott              | 6,831,044 B2 | 12/2004 | Constien            |
| 6,069,313 A           | 5/2000           | Kay                | 6,883,611 B2 | 4/2005  | Smith et al.        |
| 6,076,600 A           | 6/2000           | Vick, Jr. et al.   | 6,887,297 B2 | 5/2005  | Winter et al.       |
| 6,079,496 A           | 6/2000           | Hirth              | 6,896,049 B2 | 5/2005  | Moyses              |
| 6,085,837 A           | 7/2000           | Massinon et al.    | 6,896,061 B2 | 5/2005  | Hriscu et al.       |
| 6,095,247 A           | 8/2000           | Streich et al.     | 6,899,176 B2 | 5/2005  | Hailey, Jr. et al.  |
| 6,119,783 A           | 9/2000           | Parker et al.      | 6,899,777 B2 | 5/2005  | Vaidyanathan et al. |
| 6,142,237 A           | 11/2000          | Christmas et al.   | 6,908,516 B2 | 6/2005  | Hehmann et al.      |
| 6,161,622 A           | 12/2000          | Robb               | 6,913,827 B2 | 7/2005  | George et al.       |
| 6,167,970 B1          | 1/2001           | Stout et al.       | 6,926,086 B2 | 8/2005  | Patterson et al.    |
| 6,170,583 B1          | 1/2001           | Boyce              | 6,932,159 B2 | 8/2005  | Hovem               |
| 6,173,779 B1          | 1/2001           | Smith              | 6,939,388 B2 | 9/2005  | Angeliu             |
| 6,189,616 B1          | 2/2001           | Gano et al.        | 6,951,331 B2 | 10/2005 | Haughom et al.      |
| 6,189,618 B1          | 2/2001           | Beeman et al.      | 6,959,759 B2 | 11/2005 | Doane et al.        |
| 6,213,202 B1          | 4/2001           | Read, Jr.          | 6,973,970 B2 | 12/2005 | Johnston et al.     |
| 6,220,350 B1          | 4/2001           | Brothers et al.    | 6,973,973 B2 | 12/2005 | Howard et al.       |
| 6,228,904 B1          | 5/2001           | Yadav et al.       | 6,983,796 B2 | 1/2006  | Bayne et al.        |
| 6,237,688 B1          | 5/2001           | Burleson et al.    | 6,986,390 B2 | 1/2006  | Doane et al.        |
| 6,238,280 B1          | 5/2001           | Ritt et al.        | 7,013,989 B2 | 3/2006  | Hammond et al.      |
| 6,241,021 B1          | 6/2001           | Bowling            | 7,013,998 B2 | 3/2006  | Ray et al.          |
| 6,248,399 B1          | 6/2001           | Hehmann            | 7,017,664 B2 | 3/2006  | Walker et al.       |
| 6,250,392 B1          | 6/2001           | Muth               | 7,017,677 B2 | 3/2006  | Keshavan et al.     |
| 6,261,432 B1          | 7/2001           | Huber et al.       | 7,021,389 B2 | 4/2006  | Bishop et al.       |
| 6,273,187 B1          | 8/2001           | Voisin, Jr. et al. | 7,025,146 B2 | 4/2006  | King et al.         |
| 6,276,452 B1          | 8/2001           | Davis et al.       | 7,028,778 B2 | 4/2006  | Krywitsky           |
| 6,276,457 B1          | 8/2001           | Moffatt et al.     | 7,044,230 B2 | 5/2006  | Starr et al.        |
| 6,279,656 B1          | 8/2001           | Sinclair et al.    | 7,049,272 B2 | 5/2006  | Sinclair et al.     |
| 6,287,445 B1          | 9/2001           | Lashmore et al.    | 7,051,805 B2 | 5/2006  | Doane et al.        |
| 6,302,205 B1          | 10/2001          | Ryll               | 7,059,410 B2 | 6/2006  | Bousche et al.      |
| 6,315,041 B1          | 11/2001          | Carlisle et al.    | 7,090,027 B1 | 8/2006  | Williams            |
| 6,315,050 B2          | 11/2001          | Vaynshteyn et al.  | 7,093,664 B2 | 8/2006  | Todd et al.         |
| 6,325,148 B1          | 12/2001          | Trahan et al.      | 7,096,945 B2 | 8/2006  | Richards et al.     |
| 6,328,110 B1          | 12/2001          | Joubert            | 7,096,946 B2 | 8/2006  | Jasser et al.       |
| 6,341,653 B1          | 1/2002           | Firmaniuk et al.   | 7,097,906 B2 | 8/2006  | Gardner             |
| 6,341,747 B1          | 1/2002           | Schmidt et al.     | 7,108,080 B2 | 9/2006  | Tessari et al.      |

| (56)                  | References Cited |                          |                 |         |                     |  |
|-----------------------|------------------|--------------------------|-----------------|---------|---------------------|--|
| U.S. PATENT DOCUMENTS |                  |                          |                 |         |                     |  |
| 7,111,682 B2          | 9/2006           | Blaisdell                | 7,699,101 B2    | 4/2010  | Fripp et al.        |  |
| 7,141,207 B2          | 11/2006          | Jandeska, Jr. et al.     | 7,703,510 B2    | 4/2010  | Xu                  |  |
| 7,150,326 B2          | 12/2006          | Bishop et al.            | 7,703,511 B2    | 4/2010  | Buyers et al.       |  |
| 7,163,066 B2          | 1/2007           | Lehr                     | 7,708,078 B2    | 5/2010  | Stoesz              |  |
| 7,168,494 B2          | 1/2007           | Starr et al.             | 7,709,421 B2    | 5/2010  | Jones et al.        |  |
| 7,174,963 B2          | 2/2007           | Bertelsen                | 7,712,541 B2    | 5/2010  | Loretz et al.       |  |
| 7,182,135 B2          | 2/2007           | Szarka                   | 7,723,272 B2    | 5/2010  | Crews et al.        |  |
| 7,188,559 B1          | 3/2007           | Vecchio                  | 7,726,406 B2    | 6/2010  | Xu                  |  |
| 7,210,527 B2          | 5/2007           | Walker et al.            | 7,735,578 B2    | 6/2010  | Loehr et al.        |  |
| 7,210,533 B2          | 5/2007           | Starr et al.             | 7,752,971 B2    | 7/2010  | Loehr               |  |
| 7,234,530 B2          | 6/2007           | Gass                     | 7,757,773 B2    | 7/2010  | Rytlewski           |  |
| 7,250,188 B2          | 7/2007           | Dodelet et al.           | 7,762,342 B2    | 7/2010  | Richard et al.      |  |
| 7,252,162 B2          | 8/2007           | Akinlade et al.          | 7,770,652 B2    | 8/2010  | Barnett             |  |
| 7,255,172 B2          | 8/2007           | Johnson                  | 7,775,284 B2    | 8/2010  | Richards et al.     |  |
| 7,255,178 B2          | 8/2007           | Slup et al.              | 7,775,285 B2    | 8/2010  | Surjaatmadja et al. |  |
| 7,264,060 B2          | 9/2007           | Wills                    | 7,775,286 B2    | 8/2010  | Duphorne            |  |
| 7,267,172 B2          | 9/2007           | Hofman                   | 7,784,543 B2    | 8/2010  | Johnson             |  |
| 7,267,178 B2          | 9/2007           | Krywitsky                | 7,793,714 B2    | 9/2010  | Johnson             |  |
| 7,270,186 B2          | 9/2007           | Johnson                  | 7,798,225 B2    | 9/2010  | Giroux et al.       |  |
| 7,287,592 B2          | 10/2007          | Surjaatmadja et al.      | 7,798,226 B2    | 9/2010  | Themig              |  |
| 7,311,152 B2          | 12/2007          | Howard et al.            | 7,798,236 B2    | 9/2010  | McKeachnie et al.   |  |
| 7,316,274 B2          | 1/2008           | Xu et al.                | 7,806,189 B2    | 10/2010 | Frazier             |  |
| 7,320,365 B2          | 1/2008           | Pia                      | 7,806,192 B2    | 10/2010 | Foster et al.       |  |
| 7,322,412 B2          | 1/2008           | Badalamenti et al.       | 7,810,553 B2    | 10/2010 | Cruickshank et al.  |  |
| 7,322,417 B2          | 1/2008           | Rytlewski et al.         | 7,810,567 B2    | 10/2010 | Daniels et al.      |  |
| 7,325,617 B2          | 2/2008           | Murray                   | 7,819,198 B2    | 10/2010 | Birkhead et al.     |  |
| 7,328,750 B2          | 2/2008           | Swor et al.              | 7,828,055 B2    | 11/2010 | Willauer et al.     |  |
| 7,331,388 B2          | 2/2008           | Vilela et al.            | 7,833,944 B2    | 11/2010 | Munoz et al.        |  |
| 7,337,854 B2          | 3/2008           | Horn et al.              | 7,849,927 B2    | 12/2010 | Herrera             |  |
| 7,346,456 B2          | 3/2008           | Le Bemadjel              | 7,855,168 B2    | 12/2010 | Fuller et al.       |  |
| 7,350,582 B2          | 4/2008           | McKeachnie et al.        | 7,861,779 B2    | 1/2011  | Vestavik            |  |
| 7,353,879 B2          | 4/2008           | Todd et al.              | 7,861,781 B2    | 1/2011  | D'Arcy              |  |
| 7,360,593 B2          | 4/2008           | Constien                 | 7,874,365 B2    | 1/2011  | East, Jr. et al.    |  |
| 7,360,597 B2          | 4/2008           | Blaisdell                | 7,878,253 B2    | 2/2011  | Stowe et al.        |  |
| 7,363,970 B2          | 4/2008           | Corre et al.             | 7,896,091 B2    | 3/2011  | Williamson et al.   |  |
| 7,384,443 B2          | 6/2008           | Mirchandani              | 7,897,063 B1    | 3/2011  | Perry et al.        |  |
| 7,387,158 B2          | 6/2008           | Murray et al.            | 7,900,696 B1    | 3/2011  | Nish et al.         |  |
| 7,387,165 B2          | 6/2008           | Lopez de Cardenas et al. | 7,900,703 B2    | 3/2011  | Clark et al.        |  |
| 7,392,841 B2          | 7/2008           | Murray et al.            | 7,909,096 B2    | 3/2011  | Clark et al.        |  |
| 7,401,648 B2          | 7/2008           | Richard                  | 7,909,104 B2    | 3/2011  | Bjorgum             |  |
| 7,416,029 B2          | 8/2008           | Telfer et al.            | 7,909,110 B2    | 3/2011  | Sharma et al.       |  |
| 7,422,058 B2          | 9/2008           | O'Malley                 | 7,909,115 B2    | 3/2011  | Grove et al.        |  |
| 7,426,964 B2          | 9/2008           | Lynde et al.             | 7,913,765 B2    | 3/2011  | Crow et al.         |  |
| 7,441,596 B2          | 10/2008          | Wood et al.              | 7,931,093 B2    | 4/2011  | Foster et al.       |  |
| 7,445,049 B2          | 11/2008          | Howard et al.            | 7,938,191 B2    | 5/2011  | Vaidya              |  |
| 7,451,815 B2          | 11/2008          | Hailey, Jr.              | 7,946,335 B2    | 5/2011  | Bewlay et al.       |  |
| 7,451,817 B2          | 11/2008          | Reddy et al.             | 7,946,340 B2    | 5/2011  | Surjaatmadja et al. |  |
| 7,461,699 B2          | 12/2008          | Richard et al.           | 7,958,940 B2    | 6/2011  | Jameson             |  |
| 7,464,764 B2          | 12/2008          | Xu                       | 7,963,331 B2    | 6/2011  | Surjaatmadja et al. |  |
| 7,472,750 B2          | 1/2009           | Walker et al.            | 7,963,340 B2    | 6/2011  | Gramstad et al.     |  |
| 7,478,676 B2          | 1/2009           | East, Jr. et al.         | 7,963,342 B2    | 6/2011  | George              |  |
| 7,503,390 B2          | 3/2009           | Gomez                    | 7,980,300 B2    | 7/2011  | Roberts et al.      |  |
| 7,503,399 B2          | 3/2009           | Badalamenti et al.       | 7,987,906 B1    | 8/2011  | Troy                |  |
| 7,509,993 B1          | 3/2009           | Turng et al.             | 7,992,763 B2    | 8/2011  | Vecchio et al.      |  |
| 7,510,018 B2          | 3/2009           | Williamson et al.        | 8,020,619 B1    | 9/2011  | Robertson et al.    |  |
| 7,513,311 B2          | 4/2009           | Gramstad et al.          | 8,020,620 B2    | 9/2011  | Daniels et al.      |  |
| 7,527,103 B2          | 5/2009           | Huang et al.             | 8,025,104 B2    | 9/2011  | Cooke, Jr.          |  |
| 7,537,825 B1          | 5/2009           | Wardle et al.            | 8,028,767 B2    | 10/2011 | Radford et al.      |  |
| 7,552,777 B2          | 6/2009           | Murray et al.            | 8,033,331 B2    | 10/2011 | Themig              |  |
| 7,552,779 B2          | 6/2009           | Murray                   | 8,039,422 B1    | 10/2011 | Al-Zahrani          |  |
| 7,559,357 B2          | 7/2009           | Clem                     | 8,056,628 B2    | 11/2011 | Whitsitt et al.     |  |
| 7,575,062 B2          | 8/2009           | East, Jr.                | 8,056,638 B2    | 11/2011 | Clayton et al.      |  |
| 7,579,087 B2          | 8/2009           | Maloney et al.           | 8,109,340 B2    | 2/2012  | Doane et al.        |  |
| 7,591,318 B2          | 9/2009           | Tilghman                 | 8,127,856 B1    | 3/2012  | Nish et al.         |  |
| 7,600,572 B2          | 10/2009          | Slup et al.              | 8,153,052 B2    | 4/2012  | Jackson et al.      |  |
| 7,604,049 B2          | 10/2009          | Vaidya et al.            | 8,163,060 B2    | 4/2012  | Imanishi et al.     |  |
| 7,604,055 B2          | 10/2009          | Richard et al.           | 8,211,247 B2    | 7/2012  | Marya et al.        |  |
| 7,617,871 B2          | 11/2009          | Surjaatmadja et al.      | 8,226,740 B2    | 7/2012  | Chaumonnot et al.   |  |
| 7,635,023 B2          | 12/2009          | Goldberg et al.          | 8,230,731 B2    | 7/2012  | Dyer et al.         |  |
| 7,640,988 B2          | 1/2010           | Phi et al.               | 8,231,947 B2    | 7/2012  | Vaidya et al.       |  |
| 7,661,480 B2          | 2/2010           | Al-Anazi                 | 8,276,670 B2    | 10/2012 | Patel               |  |
| 7,661,481 B2          | 2/2010           | Todd et al.              | 8,277,974 B2    | 10/2012 | Kumar et al.        |  |
| 7,665,537 B2          | 2/2010           | Patel et al.             | 8,297,364 B2    | 10/2012 | Agrawal et al.      |  |
| 7,686,082 B2          | 3/2010           | Marsh                    | 8,327,931 B2    | 12/2012 | Agrawal et al.      |  |
| 7,690,436 B2          | 4/2010           | Turley et al.            | 8,403,037 B2    | 3/2013  | Agrawal et al.      |  |
|                       |                  |                          | 8,425,651 B2    | 4/2013  | Xu et al.           |  |
|                       |                  |                          | 2001/0045288 A1 | 11/2001 | Russell             |  |
|                       |                  |                          | 2001/0045288 A1 | 11/2001 | Allamon et al.      |  |
|                       |                  |                          | 2002/0000319 A1 | 1/2002  | Brunet              |  |

| (56)                  | References Cited |                        |                 |         |                        |  |  |
|-----------------------|------------------|------------------------|-----------------|---------|------------------------|--|--|
| U.S. PATENT DOCUMENTS |                  |                        |                 |         |                        |  |  |
| 2002/0007948 A1       | 1/2002           | Bayne et al.           | 2006/0283592 A1 | 12/2006 | Sierra et al.          |  |  |
| 2002/0014268 A1       | 2/2002           | Vann                   | 2007/0017674 A1 | 1/2007  | Blaisdell              |  |  |
| 2002/0066572 A1       | 6/2002           | Muth                   | 2007/0017675 A1 | 1/2007  | Hammami                |  |  |
| 2002/0104616 A1       | 8/2002           | De et al.              | 2007/0029082 A1 | 2/2007  | Giroux et al.          |  |  |
| 2002/0136904 A1       | 9/2002           | Glass et al.           | 2007/0039741 A1 | 2/2007  | Hailey                 |  |  |
| 2002/0162661 A1       | 11/2002          | Krauss et al.          | 2007/0044958 A1 | 3/2007  | Rytlewski et al.       |  |  |
| 2003/0037925 A1       | 2/2003           | Walker et al.          | 2007/0044966 A1 | 3/2007  | Davies et al.          |  |  |
| 2003/0060374 A1       | 3/2003           | Cooke, Jr.             | 2007/0051521 A1 | 3/2007  | Fike et al.            |  |  |
| 2003/0075326 A1       | 4/2003           | Ebinger                | 2007/0053785 A1 | 3/2007  | Hetz et al.            |  |  |
| 2003/0104147 A1       | 6/2003           | Bretschneider et al.   | 2007/0054101 A1 | 3/2007  | Sigalas et al.         |  |  |
| 2003/0111728 A1       | 6/2003           | Thai et al.            | 2007/0057415 A1 | 3/2007  | Katagiri et al.        |  |  |
| 2003/0127013 A1       | 7/2003           | Zavitsanos et al.      | 2007/0062644 A1 | 3/2007  | Nakamura et al.        |  |  |
| 2003/0141060 A1       | 7/2003           | Hailey et al.          | 2007/0074601 A1 | 4/2007  | Hong et al.            |  |  |
| 2003/0141061 A1       | 7/2003           | Hailey et al.          | 2007/0074873 A1 | 4/2007  | McKeachnie et al.      |  |  |
| 2003/0141079 A1       | 7/2003           | Doane et al.           | 2007/0102199 A1 | 5/2007  | Smith et al.           |  |  |
| 2003/0150614 A1       | 8/2003           | Brown et al.           | 2007/0107899 A1 | 5/2007  | Werner et al.          |  |  |
| 2003/0155114 A1       | 8/2003           | Pedersen et al.        | 2007/0107908 A1 | 5/2007  | Vaidya et al.          |  |  |
| 2003/0155115 A1       | 8/2003           | Pedersen et al.        | 2007/0108060 A1 | 5/2007  | Park                   |  |  |
| 2003/0159828 A1       | 8/2003           | Howard et al.          | 2007/0119600 A1 | 5/2007  | Slup et al.            |  |  |
| 2003/0164237 A1       | 9/2003           | Butterfield            | 2007/0131912 A1 | 6/2007  | Simone et al.          |  |  |
| 2003/0183391 A1       | 10/2003          | Hriscu et al.          | 2007/0151009 A1 | 7/2007  | Conrad, III et al.     |  |  |
| 2004/0005483 A1       | 1/2004           | Lin                    | 2007/0151769 A1 | 7/2007  | Slutz et al.           |  |  |
| 2004/0020832 A1       | 2/2004           | Richards et al.        | 2007/0169935 A1 | 7/2007  | Akbar et al.           |  |  |
| 2004/0031605 A1       | 2/2004           | Mickey                 | 2007/0181224 A1 | 8/2007  | Marya et al.           |  |  |
| 2004/0045723 A1       | 3/2004           | Slup et al.            | 2007/0185655 A1 | 8/2007  | Le Bemadjiel           |  |  |
| 2004/0055758 A1       | 3/2004           | Brezinski et al.       | 2007/0187095 A1 | 8/2007  | Walker et al.          |  |  |
| 2004/0089449 A1       | 5/2004           | Walton et al.          | 2007/0221373 A1 | 9/2007  | Murray                 |  |  |
| 2004/0154806 A1       | 8/2004           | Bode et al.            | 2007/0221384 A1 | 9/2007  | Murray                 |  |  |
| 2004/0159428 A1       | 8/2004           | Hammond et al.         | 2007/0259994 A1 | 11/2007 | Tour et al.            |  |  |
| 2004/0182583 A1       | 9/2004           | Doane et al.           | 2007/0261862 A1 | 11/2007 | Murray                 |  |  |
| 2004/0231845 A1       | 11/2004          | Cooke, Jr.             | 2007/0272411 A1 | 11/2007 | Lopez De Cerdas et al. |  |  |
| 2004/0256109 A1       | 12/2004          | Johnson                | 2007/0272413 A1 | 11/2007 | Rytlewski et al.       |  |  |
| 2004/0256157 A1       | 12/2004          | Tessari et al.         | 2007/0277979 A1 | 12/2007 | Todd et al.            |  |  |
| 2004/0261993 A1       | 12/2004          | Nguyen                 | 2007/0284109 A1 | 12/2007 | East et al.            |  |  |
| 2005/0034876 A1       | 2/2005           | Doane et al.           | 2007/0284112 A1 | 12/2007 | Magne et al.           |  |  |
| 2005/0051329 A1       | 3/2005           | Blaisdell              | 2007/0299510 A1 | 12/2007 | Venkatraman et al.     |  |  |
| 2005/0064247 A1       | 3/2005           | Sane et al.            | 2008/0011473 A1 | 1/2008  | Wood et al.            |  |  |
| 2005/0069449 A1       | 3/2005           | Jackson et al.         | 2008/0020923 A1 | 1/2008  | Debe et al.            |  |  |
| 2005/0102255 A1       | 5/2005           | Bultman                | 2008/0047707 A1 | 2/2008  | Boney et al.           |  |  |
| 2005/0106316 A1       | 5/2005           | Rigney et al.          | 2008/0060810 A9 | 3/2008  | Nguyen et al.          |  |  |
| 2005/0126334 A1       | 6/2005           | Mirchandani            | 2008/0066923 A1 | 3/2008  | Xu                     |  |  |
| 2005/0161212 A1       | 7/2005           | Leismer et al.         | 2008/0066924 A1 | 3/2008  | Xu                     |  |  |
| 2005/0161224 A1       | 7/2005           | Starr et al.           | 2008/0072705 A1 | 3/2008  | Chaumonnot et al.      |  |  |
| 2005/0165149 A1       | 7/2005           | Chanak et al.          | 2008/0078553 A1 | 4/2008  | George                 |  |  |
| 2005/0194143 A1       | 9/2005           | Xu et al.              | 2008/0081866 A1 | 4/2008  | Gong et al.            |  |  |
| 2005/0199401 A1       | 9/2005           | Patel et al.           | 2008/0099209 A1 | 5/2008  | Loretz et al.          |  |  |
| 2005/0205264 A1       | 9/2005           | Starr et al.           | 2008/0105438 A1 | 5/2008  | Jordan et al.          |  |  |
| 2005/0205265 A1       | 9/2005           | Todd et al.            | 2008/0115932 A1 | 5/2008  | Cooke                  |  |  |
| 2005/0205266 A1       | 9/2005           | Todd et al.            | 2008/0121390 A1 | 5/2008  | O'Malley et al.        |  |  |
| 2005/0241824 A1       | 11/2005          | Burris, II et al.      | 2008/0121436 A1 | 5/2008  | Slay et al.            |  |  |
| 2005/0241825 A1       | 11/2005          | Burris, II et al.      | 2008/0127475 A1 | 6/2008  | Griffo                 |  |  |
| 2005/0257936 A1       | 11/2005          | Lehr                   | 2008/0135249 A1 | 6/2008  | Fripp et al.           |  |  |
| 2005/0279501 A1       | 12/2005          | Surjaatmadja et al.    | 2008/0149325 A1 | 6/2008  | Crawford               |  |  |
| 2006/0012087 A1       | 1/2006           | Matsuda et al.         | 2008/0149345 A1 | 6/2008  | Bicerano               |  |  |
| 2006/0045787 A1       | 3/2006           | Jandeska et al.        | 2008/0149351 A1 | 6/2008  | Marya et al.           |  |  |
| 2006/0057479 A1       | 3/2006           | Niimi et al.           | 2008/0169105 A1 | 7/2008  | Williamson et al.      |  |  |
| 2006/0081378 A1       | 4/2006           | Howard et al.          | 2008/0179060 A1 | 7/2008  | Surjaatmadja et al.    |  |  |
| 2006/0102871 A1       | 5/2006           | Wang                   | 2008/0179104 A1 | 7/2008  | Zhang et al.           |  |  |
| 2006/0108114 A1       | 5/2006           | Johnson                | 2008/0202764 A1 | 8/2008  | Clayton et al.         |  |  |
| 2006/0108126 A1       | 5/2006           | Horn et al.            | 2008/0202814 A1 | 8/2008  | Lyons et al.           |  |  |
| 2006/0110615 A1       | 5/2006           | Karim et al.           | 2008/0210473 A1 | 9/2008  | Zhang et al.           |  |  |
| 2006/0116696 A1       | 6/2006           | Odermatt et al.        | 2008/0216383 A1 | 9/2008  | Pierick et al.         |  |  |
| 2006/0124310 A1       | 6/2006           | Lopez de Cerdas et al. | 2008/0223586 A1 | 9/2008  | Barnett                |  |  |
| 2006/0124312 A1       | 6/2006           | Rytlewski et al.       | 2008/0223587 A1 | 9/2008  | Cherewyk               |  |  |
| 2006/0131011 A1       | 6/2006           | Lynde et al.           | 2008/0236829 A1 | 10/2008 | Lynde                  |  |  |
| 2006/0131031 A1       | 6/2006           | McKeachnie et al.      | 2008/0248205 A1 | 10/2008 | Blanchet et al.        |  |  |
| 2006/0131081 A1       | 6/2006           | Mirchandani et al.     | 2008/0248413 A1 | 10/2008 | Ishii et al.           |  |  |
| 2006/0144515 A1       | 7/2006           | Tada et al.            | 2008/0277109 A1 | 11/2008 | Vaidya                 |  |  |
| 2006/0150770 A1       | 7/2006           | Freim                  | 2008/0277980 A1 | 11/2008 | Koda et al.            |  |  |
| 2006/0151178 A1       | 7/2006           | Howard et al.          | 2008/0282924 A1 | 11/2008 | Saenger et al.         |  |  |
| 2006/0162927 A1       | 7/2006           | Walker et al.          | 2008/0296024 A1 | 12/2008 | Huang et al.           |  |  |
| 2006/0169453 A1       | 8/2006           | Savery et al.          | 2008/0314581 A1 | 12/2008 | Brown                  |  |  |
| 2006/0207763 A1       | 9/2006           | Hofman et al.          | 2008/0314588 A1 | 12/2008 | Langlais et al.        |  |  |
| 2006/0213670 A1       | 9/2006           | Bishop et al.          | 2009/0038858 A1 | 2/2009  | Griffo et al.          |  |  |
| 2006/0231253 A1       | 10/2006          | Vilela et al.          | 2009/0044946 A1 | 2/2009  | Schasteen et al.       |  |  |
|                       |                  |                        | 2009/0044949 A1 | 2/2009  | King et al.            |  |  |
|                       |                  |                        | 2009/0050334 A1 | 2/2009  | Marya et al.           |  |  |
|                       |                  |                        | 2009/0056934 A1 | 3/2009  | Xu                     |  |  |
|                       |                  |                        | 2009/0065216 A1 | 3/2009  | Frazier                |  |  |

(56)

## References Cited

## U.S. PATENT DOCUMENTS

|                 |         |                          |                                                                                                                                                                                               |               |                     |
|-----------------|---------|--------------------------|-----------------------------------------------------------------------------------------------------------------------------------------------------------------------------------------------|---------------|---------------------|
| 2009/0084553 A1 | 4/2009  | Rytlewski et al.         | 2011/0135530 A1                                                                                                                                                                               | 6/2011        | Xu et al.           |
| 2009/0084556 A1 | 4/2009  | Richards et al.          | 2011/0135805 A1                                                                                                                                                                               | 6/2011        | Doucet et al.       |
| 2009/0084600 A1 | 4/2009  | Severance                | 2011/0135953 A1                                                                                                                                                                               | 6/2011        | Xu et al.           |
| 2009/0090440 A1 | 4/2009  | Kellett                  | 2011/0136707 A1                                                                                                                                                                               | 6/2011        | Xu et al.           |
| 2009/0107684 A1 | 4/2009  | Cooke, Jr.               | 2011/0139465 A1                                                                                                                                                                               | 6/2011        | Tibbles et al.      |
| 2009/0114382 A1 | 5/2009  | Grove et al.             | 2011/0147014 A1                                                                                                                                                                               | 6/2011        | Chen et al.         |
| 2009/0145666 A1 | 6/2009  | Radford et al.           | 2011/0186306 A1                                                                                                                                                                               | 8/2011        | Marya et al.        |
| 2009/0151949 A1 | 6/2009  | Marya et al.             | 2011/0214881 A1                                                                                                                                                                               | 9/2011        | Newton              |
| 2009/0152009 A1 | 6/2009  | Slay et al.              | 2011/0247833 A1                                                                                                                                                                               | 10/2011       | Todd et al.         |
| 2009/0155616 A1 | 6/2009  | Thamida                  | 2011/0253387 A1                                                                                                                                                                               | 10/2011       | Ervin               |
| 2009/0159289 A1 | 6/2009  | Avant et al.             | 2011/0256356 A1                                                                                                                                                                               | 10/2011       | Tomantschger et al. |
| 2009/0178808 A1 | 7/2009  | Williamson et al.        | 2011/0259610 A1                                                                                                                                                                               | 10/2011       | Shkurti et al.      |
| 2009/0194273 A1 | 8/2009  | Surjaatmadja et al.      | 2011/0277987 A1                                                                                                                                                                               | 11/2011       | Frazier             |
| 2009/0205841 A1 | 8/2009  | Kluge et al.             | 2011/0277989 A1                                                                                                                                                                               | 11/2011       | Frazier             |
| 2009/0226340 A1 | 9/2009  | Marya                    | 2011/0284232 A1                                                                                                                                                                               | 11/2011       | Huang               |
| 2009/0226704 A1 | 9/2009  | Kauppinen et al.         | 2011/0284240 A1                                                                                                                                                                               | 11/2011       | Chen et al.         |
| 2009/0242202 A1 | 10/2009 | Risppler et al.          | 2011/0284243 A1                                                                                                                                                                               | 11/2011       | Frazier             |
| 2009/0242208 A1 | 10/2009 | Bolding                  | 2011/0300403 A1                                                                                                                                                                               | 12/2011       | Vecchio et al.      |
| 2009/0242214 A1 | 10/2009 | Foster et al.            | 2012/0067426 A1                                                                                                                                                                               | 3/2012        | Soni et al.         |
| 2009/0255667 A1 | 10/2009 | Clem et al.              | 2012/0103135 A1                                                                                                                                                                               | 5/2012        | Xu et al.           |
| 2009/0255684 A1 | 10/2009 | Bolding                  | 2012/0107590 A1                                                                                                                                                                               | 5/2012        | Xu et al.           |
| 2009/0255686 A1 | 10/2009 | Richard                  | 2012/0118583 A1                                                                                                                                                                               | 5/2012        | Johnson et al.      |
| 2009/0260817 A1 | 10/2009 | Gambier et al.           | 2012/0130470 A1                                                                                                                                                                               | 5/2012        | Agnew               |
| 2009/0266548 A1 | 10/2009 | Olsen et al.             | 2012/0145389 A1                                                                                                                                                                               | 6/2012        | Fitzpatrick, Jr.    |
| 2009/0272544 A1 | 11/2009 | Giroux et al.            | 2012/0168152 A1                                                                                                                                                                               | 7/2012        | Casciaro et al.     |
| 2009/0283270 A1 | 11/2009 | Langeslag                | 2012/0211239 A1                                                                                                                                                                               | 8/2012        | Kritzler et al.     |
| 2009/0293672 A1 | 12/2009 | Mirchandani et al.       | 2012/0267101 A1                                                                                                                                                                               | 10/2012       | Cooke               |
| 2009/0301730 A1 | 12/2009 | Gweily                   | 2012/0292053 A1                                                                                                                                                                               | 11/2012       | Xu et al.           |
| 2009/0305131 A1 | 12/2009 | Kumar et al.             | 2012/0318513 A1                                                                                                                                                                               | 12/2012       | Mazyar et al.       |
| 2009/0308588 A1 | 12/2009 | Howell et al.            | 2013/0004847 A1                                                                                                                                                                               | 1/2013        | Kumar et al.        |
| 2009/0317556 A1 | 12/2009 | Macary                   | 2013/0025409 A1                                                                                                                                                                               | 1/2013        | Xu                  |
| 2010/0003536 A1 | 1/2010  | Smith et al.             | 2013/0032357 A1                                                                                                                                                                               | 2/2013        | Mazyar et al.       |
| 2010/0012385 A1 | 1/2010  | Drivdahl et al.          | 2013/0048304 A1                                                                                                                                                                               | 2/2013        | Agrawal et al.      |
| 2010/0015002 A1 | 1/2010  | Barrera et al.           | 2013/0052472 A1                                                                                                                                                                               | 2/2013        | Xu                  |
| 2010/0015469 A1 | 1/2010  | Romanowski et al.        | 2013/0081814 A1                                                                                                                                                                               | 4/2013        | Gaudette et al.     |
| 2010/0025255 A1 | 2/2010  | Su et al.                | 2013/0105159 A1                                                                                                                                                                               | 5/2013        | Alvarez             |
| 2010/0032151 A1 | 2/2010  | Duphorne                 | 2013/0126190 A1                                                                                                                                                                               | 5/2013        | Mazyar et al.       |
| 2010/0040180 A1 | 2/2010  | Kim et al.               | 2013/0133897 A1                                                                                                                                                                               | 5/2013        | Baihly et al.       |
| 2010/0044041 A1 | 2/2010  | Smith et al.             | 2013/0146144 A1                                                                                                                                                                               | 6/2013        | Joseph et al.       |
| 2010/0051278 A1 | 3/2010  | Mytopher et al.          | 2013/0146302 A1                                                                                                                                                                               | 6/2013        | Gaudette et al.     |
| 2010/0055491 A1 | 3/2010  | Vecchio et al.           | 2013/0186626 A1                                                                                                                                                                               | 7/2013        | Aitken et al.       |
| 2010/0055492 A1 | 3/2010  | Barsoum et al.           | 2013/0240203 A1                                                                                                                                                                               | 9/2013        | Frazier             |
| 2010/0089583 A1 | 4/2010  | Xu et al.                | 2013/0327540 A1                                                                                                                                                                               | 12/2013       | Hamid et al.        |
| 2010/0089587 A1 | 4/2010  | Stout                    | 2014/0116711 A1                                                                                                                                                                               | 5/2014        | Tang et al.         |
| 2010/0101803 A1 | 4/2010  | Clayton et al.           | FOREIGN PATENT DOCUMENTS                                                                                                                                                                      |               |                     |
| 2010/0122817 A1 | 5/2010  | Surjaatmadja et al.      | CN                                                                                                                                                                                            | 101050417 A   | 10/2007             |
| 2010/0139930 A1 | 6/2010  | Patel et al.             | CN                                                                                                                                                                                            | 101351523 A   | 1/2009              |
| 2010/0200230 A1 | 8/2010  | East, Jr. et al.         | CN                                                                                                                                                                                            | 101457321 A   | 6/2009              |
| 2010/0236793 A1 | 9/2010  | Bjorgum                  | EP                                                                                                                                                                                            | 0033625 A1    | 8/1981              |
| 2010/0236794 A1 | 9/2010  | Duan et al.              | EP                                                                                                                                                                                            | 1857570 A2    | 11/2007             |
| 2010/0243254 A1 | 9/2010  | Murphy et al.            | GB                                                                                                                                                                                            | 912956        | 12/1962             |
| 2010/0252273 A1 | 10/2010 | Duphorne                 | JP                                                                                                                                                                                            | 61067770      | 4/1986              |
| 2010/0252280 A1 | 10/2010 | Swor et al.              | JP                                                                                                                                                                                            | 754008 A      | 2/1995              |
| 2010/0270031 A1 | 10/2010 | Patel                    | JP                                                                                                                                                                                            | 8232029 A     | 9/1996              |
| 2010/0276136 A1 | 11/2010 | Evans et al.             | JP                                                                                                                                                                                            | 2000185725 A1 | 7/2000              |
| 2010/0282338 A1 | 11/2010 | Gerrard et al.           | JP                                                                                                                                                                                            | 2004225084 A  | 8/2004              |
| 2010/0282469 A1 | 11/2010 | Richard et al.           | JP                                                                                                                                                                                            | 2004225765 A  | 8/2004              |
| 2010/0294510 A1 | 11/2010 | Holmes                   | JP                                                                                                                                                                                            | 2005076052 A  | 3/2005              |
| 2010/0319870 A1 | 12/2010 | Bewlay et al.            | JP                                                                                                                                                                                            | 2010502840 A  | 1/2010              |
| 2011/0005773 A1 | 1/2011  | Dusterhoff et al.        | KR                                                                                                                                                                                            | 950014350 B1  | 11/1995             |
| 2011/0036592 A1 | 2/2011  | Fay                      | WO                                                                                                                                                                                            | 9947726       | 9/1999              |
| 2011/0048743 A1 | 3/2011  | Stafford et al.          | WO                                                                                                                                                                                            | 2008034042 A3 | 3/2008              |
| 2011/0056692 A1 | 3/2011  | Lopez de Cardenas et al. | WO                                                                                                                                                                                            | 2008057045 A1 | 5/2008              |
| 2011/0056702 A1 | 3/2011  | Sharma et al.            | WO                                                                                                                                                                                            | 2008079485 A2 | 7/2008              |
| 2011/0067872 A1 | 3/2011  | Agrawal                  | WO                                                                                                                                                                                            | 2008079777 A3 | 7/2008              |
| 2011/0067889 A1 | 3/2011  | Marya et al.             | WO                                                                                                                                                                                            | 2009079745 A1 | 7/2009              |
| 2011/0067890 A1 | 3/2011  | Themig                   | WO                                                                                                                                                                                            | 2011071902 A2 | 6/2011              |
| 2011/0094406 A1 | 4/2011  | Marya et al.             | WO                                                                                                                                                                                            | 2011071910 A3 | 6/2011              |
| 2011/0100643 A1 | 5/2011  | Themig et al.            | WO                                                                                                                                                                                            | 2012174101 A2 | 12/2012             |
| 2011/0127044 A1 | 6/2011  | Radford et al.           | WO                                                                                                                                                                                            | 2013053057 A1 | 4/2013              |
| 2011/0132143 A1 | 6/2011  | Xu et al.                | WO                                                                                                                                                                                            | 2013078031 A1 | 5/2013              |
| 2011/0132612 A1 | 6/2011  | Agrawal et al.           | OTHER PUBLICATIONS                                                                                                                                                                            |               |                     |
| 2011/0132619 A1 | 6/2011  | Agrawal et al.           | International Search Report and Written Opinion of the International Searching Authority mailed on Feb. 19, 2013, for International Application No. PCT/US2012/053342 filed on Aug. 31, 2012. |               |                     |
| 2011/0132620 A1 | 6/2011  | Agrawal et al.           |                                                                                                                                                                                               |               |                     |
| 2011/0132621 A1 | 6/2011  | Agrawal et al.           |                                                                                                                                                                                               |               |                     |

(56)

## References Cited

## OTHER PUBLICATIONS

- International Search Report and Written Opinion of the International Searching Authority mailed on Feb. 15, 2013 for International Application No. PCT/US2012/053339 filed on Aug. 31, 2012.
- International Search Report and Written Opinion of the International Searchign Authority mailed on Feb. 25, 2013 for International application No. PCT/US2012/053350 filed on Aug. 31, 2012.
- International Search Report and Written Opinion; International Application No. PCT/US2010/057763; International Filing Date: Nov. 23, 2010; Date of Mailing: Jul. 28, 2011; 10 pages.
- International Search Report and Written Opinion; International Application No. PCT/US2010/059259; International Filing Date: Dec. 7, 2010; Date of Mailing: Jun. 13, 2011; 8 pages.
- International Search Report and Written Opinion; International Application No. PCT/US2010/059265; International Filing Date: Dec. 7, 2010; Date of Mailing: Jun. 16, 2011; 8 pages.
- International Search Report and Written Opinion; International Application No. PCT/US2010/059268; International Filing Date: Dec. 7, 2010; Date of Mailing: Jun. 17, 2011; 8 pages.
- International Search Report and Written Opinion; International Application No. PCT/US20111058105; International Filing Date: Oct. 27, 2011; Date of Mailing: May 1, 2012; 8 pages.
- International Search Report and Written Opinion; International Application No. PCT/US2012/034973; International Filing Date: Apr. 25, 2012; Date of Mailing: Nov. 29, 2012; 8 pages.
- International Search Report and Written Opinion; International Application No. PCT/US2012/034978; International Filing Date: Apr. 25, 2012; Date of Mailing: Nov. 12, 2012; 9 pages.
- International Search Report and Written Opinion; International Application No. PCT/US2012/038622; International Filing Date: May 18, 2012; Date of Mailing: Dec. 6, 2012; 12 pages.
- International Search Report and Written Opinion; International Application No. PCT/US2012/044866; International Filing Date: Jun. 29, 2012; Date of Mailing: Jan. 2, 2013; 9 pages.
- International Search Report and Written Opinion; International Application No. PCT/US2012/046231; International Filing Date: Jul. 11, 2012; Date of Mailing: Jan. 29, 2013; 9 pages.
- International Search Report and Written Opinion; International Application No. PCT/US2012/049434; International Filing Date: Aug. 3, 2012; Date of Mailing: Feb. 1, 2013; 7 pages.
- International Search Report and Written Opinion; International Application No. PCT/US2014/049347; International Filing Date: Aug. 1, 2014; Date of Mailing: Nov. 24, 2014; 11 pages.
- International Search Report and Written Opinion; International Application No. PCT/US2014/054720; International Filing Date: Sep. 9, 2014; Date of Mailing: Dec. 17, 2014; 10 pages.
- Lunder et al.; "The Role of Mg17Al12 Phase in the Corrosion of Mg Alloy AZ91"; Corrosion; 45(9); pp. 741-748; (1989).
- Majumdar, et al., "Laser Surface Engineering of a Magnesium Alloy with Al + Al<sub>2</sub>O<sub>3</sub>", Surface and Coatings Technology 179 (2004) pp. 297-305.
- Mathis, "Sand Management: A Review of Approaches and Concerns", Society of Petroleum Engineers, SPE Paper No. 82240, SPE European Formation Damage Conference, The Hague, The Netherlands, May 13-14, 2003.
- Nie, "Patents of Methods to Prepare Intermetallic Matrix Composites: A Review", Recent Patents on Materials Science 2008, vol. 1, pp. 232-240.
- Pardo, et al.; "Corrosion Behaviour of Magnesium/Aluminium Alloys in 3.5 wt% NaCl"; Corrosion Science; 50; pp. 823-834; (2008).
- Rose, et al.; "The application of the polyaromatic sulfonates as tracers in geothermal reservoirs", Geothermics 30 (2001) pp. 617-640.
- Shaw, "Benefits and Application of a Surface-Controlled Sliding Sleeve for Fracturing Operations"; Society of Petroleum Engineers, SPE Paper No. 147546; Oct. 30, 2011; 8 pages.
- Shigematsu, et al., "Surface Treatment of AZ91D Magnesium Alloy by Aluminum diffusion Coating", Journal of Materials Science Letters 19, 2000, pp. 473-475.
- Singh, et al., "Extended Homogeneity Range of Intermetallic Phases in Mechanically Alloyed Mg-Al Alloys", Elsevier Sciences Ltd., Intemetallics 11, 2003, pp. 373-376.
- Song, "Recent Progress in Corrosion and Protection of Magnesium Alloys"; Advanced Engineering Materials; 7(7); pp. 563-586; (2005).
- Song, et al.; "A Possible Biodegradable Magnesium Implant Material," Advanced Engineering Materials, vol. 9, Issue 4, Apr. 2007, pp. 298-302.
- Song, et al.; "Corrosion Behaviour of AZ21, AZ501 and AZ91 in Sodium Chloride"; Corrosion Science; 40(10); pp. 1769-1791; (1998).
- Song, et al.; "Corrosion Mechanisms of Magnesium Alloys"; Advanced Engineering Materials; 1(1); pp. 11-33; (1999).
- Song, et al.; "Influence of Microstructure on the Corrosion of Diecast AZ91D"; Corrosion Science; 41; pp. 249-273; (1999).
- Song, et al.; "Understanding Magnesium Corrosion"; Advanced Engineering Materials; 5; No. 12; pp. 837-858; (2003).
- Stanley, et al.; "An Introduction to Ground-Water Tracers", Department of Hydrology and Water Resources, University of Arizona, Mar. 1985, pp. 1-219.
- Sun, et al.; "Colloidal Processing of Carbon Nanotube/Alumina Composites" Chem. Mater. 2002, 14, pp. 5169-5172.
- Vahlas, et al., "Principles and Applications of CVD Powder Technology", Materials Science and Engineering R 53 (2006) pp. 1-72.
- Vickery, et al.; "New One-Trip Multi-Zone Frac Pack System with Positive Positioning." European Petroleum Conference, Oct. 29-31, 2002, Aberdeen, UK.
- Xu, et al., "Nanostructured Material-Based Completion Tools Enhance Well Productivity"; International Petroleum Technology Conference; Conference Paper IPTC 16538; International Petroleum Technology Conference 2013; 4 pages.
- Zemel, "Tracers in the Oil Field", University of Texas at Austin, Center for Petroleum and Geosystems, Jan. 1995, Chapters 1, 2, 3, 7.
- Zeng, et al. "Progress and Challenge for Magnesium Alloys as Biomaterials", Advanced Engineering Materials, vol. 10, Issue 8, Aug. 2008, pp. B3-B14.
- Zhan, et al., "Single-wall carbon nanotubes as attractive toughening agents in alumina-based nanocomposites" Nature Materials, vol. 2., Jan. 2003, pp. 38-42.
- Zhang, et al.; "Formation of metal nanowires on suspended single-walled carbon nanotubes" Applied Physics Letter, vol. 77, No. 19 (2000), pp. 3015-3017.
- Zhang, et al.; "High Strength Nanostructured Materials and Their Oil Field Applications"; Society of Petroleum Engineers; Conference Paper SPE 157092; SPE International Oilfield Nanotechnology Conference, 2012; 6 pages.
- Zhang, et al.; "Metal Coating on Suspended Carbon Nanotubes and its Implication to Metal—Tube Interaction", Chemical Physics Letters 331 (2000) 35-41.
- Zhang, et al.; "Study on the Environmentally Friendly Anodizing of AZ91D Magnesium Alloy"; Surface and Coatings Technology: 161; pp. 36-43; (2002).
- "Optisleeve Sliding Sleeve", [online]; [retrieved on Jun. 25, 2010]; retrieved from the Internet [weatherfordcorp/WFT033159.pdf](http://weatherford.com/weatherford/groups/.../weatherfordcorp/WFT033159.pdf).
- "Reactivity series", Wikipedia, [http://en.wikipedia.org/w/index.php?title=Reactivity\\_series&printable=yes](http://en.wikipedia.org/w/index.php?title=Reactivity_series&printable=yes) downloaded on May 18, 2014. 8 pages.
- "Sliding Sleeve", Omega Completion Technology Ltd, Sep. 29, 2009, retrieved on: [www.omega-completion.com](http://www.omega-completion.com).
- Adams, et al.; "Thermal stabilities of aromatic acids as geothermal tracers", Geothermics, vol. 21, No. 3, 1992, pp. 323-339.
- Ambat, et al., "Electroless Nickel-Plating on AZ91D Magnesium Alloy: Effect of Substrate Microstructure and Plating Parameters"; Surface and Coatings Technology; 179; pp. 124-134; (2004).
- Ayman, et al.; "Effect of Consolidation and Extrusion Temperatures on Tensile Properties of Hot Extruded ZK61 Magnesium Alloy Gas Atomized Powders via Spark Plasma Sintering", Transactions of JWRI, vol. 38 (2009), No. 2, pp. 1-5.
- Baker Hughes, "Flow Control Systems," [online]; [retrieved on May 20, 2010]; retrieved from the Internet <http://www.bakerhughes.com/>

(56)

**References Cited****OTHER PUBLICATIONS**

- products-and-services/completions-and-productions/well-completions/packers-and-flow-control/flow-control-systems.
- Baker Oil Tools, "Baker Oil Tools Introduces Revolutionary Sand Control Completion Technology," May 2, 2005.
- Bastow, et al., "Clustering and formation of nano-precipitates in dilute aluminum and magnesium alloys", Materials Science and Engineering, 2003, C23, 757-762.
- Bercegeay, et al., "A One-Trip Gravel Packing System"; Society of Petroleum Engineers, Offshore Technology Conference, SPE Paper No. 4771; Feb. 7-8, 1974.
- Birbilis, et al., "Exploring Corrosion Protection of Mg Via Ionic Liquid Pretreatment", Surface & Coatings Technology; 201, pp. 4496-4504, (2007).
- Bybee, "One-Trip Completion System Eliminates Perforations," Completions Today, Sep. 2007, pp. 52-53.
- Carrejo, et al., "Improving Flow Assurance in Multi-Zone Fracturing Treatments in Hydrocarbon Reservoirs with High Strength Corrodible Tripping Balls"; Society of Petroleum Engineers; SPE Paper No. 151613; Apr. 16, 2012; 6 pages.
- Christoglou, et al., "Deposition of Aluminum on Magnesium by a CVD Process", Surface and Coatings Technology 184 (2004) 149-155.
- Constantine, "Selective Production of Horizontal Openhole Completions Using ECP and Sliding Sleeve Technology," SPE Rocky Mountain Regional Meeting, May 15-18, 1999, Gillette, Wyoming.
- Curtin, et al., "CNT-reinforced ceramics and metals," Materials Today, 2004, vol. 7, pp. 44-49.
- Feng, et al., "Electroless Plating of Carbon Nanotubes with Silver" Journal of Materials Science, 39, (2004) pp. 3241-3243.
- Flahaut, et al., "Carbon Nanotube-Metal-Oxide Nanocomposites: Microstructure, Electrical Conductivity and Mechanical Properties" Acta amter. 48 (2000), pp. 3803-3812.
- Forsyth, et al.; "An Ionic Liquid Surface Treatment for Corrosion Protection of Magnesium Alloy AZ31"; Electrochem. Solid-State Lett. 2006, vol. 9, Issue 11, B52-B55.
- Galanty, et al. "Consolidation of metal powders during the extrusion process," Journal of Materials Processing Technology (2002), pp. 491-496.
- Garfield, New One-Trip Sand-Control Completion System that Eliminates Formation Damage Resulting From conventional Perforating and Gravel-Pack Operations.; SPE Annual Technical Conference and Exhibition, Oct. Sep. 12, 2005.
- Garfield, et al., "Maximizing Inflow Performance in Soft Sand Completions Using New One-trip Sand Control Liner Completion Technology", SPE European Formation Damage Conference, May 25-27, 2005.
- Goh, et al., "Development of novel carbon nanotube reinforced magnesium nanocomposites using the powder metallurgy technique", Nanotechnology 17 (2006) 7-12.
- Hermawan, et al., "Iron-manganese: new class of metallic degradable biomaterials prepared by powder metallurgy", Powder Metallurgy, vol. 51, No. 1, (2008), pp. 38-45.
- Hjortstam, et al. "Can we achieve ultra-low resistivity in carbon nanotube-based metal composites," Applied Physics a (2004), vol. 78, Issue 8, pp. 1175-1179.
- Hsiao, et al., "Anodization of AZ91D Magnesium Alloy in Silicate-Containing Electrolytes"; Surface & Coatings Technology; 199; pp. 127-134; (2005).
- Hsiao, et al., "Baking Treatment Effect on Materials Characteristics and Electrochemical Behavior of anodic Film Formed on AZ91D Magnesium Alloy"; Corrosion Science; 49; pp. 781-793; (2007).
- Hsiao, et al., "Characterization of Anodic Films Formed on AZ91D Magnesium Alloy"; Surface & Coatings Technology; 190; pp. 299-308; (2005).
- Hsiao, et al., "Effect of Heat Treatment on Anodization and Electrochemical Behavior of AZ91D Magnesium Alloy"; J. Mater Res.; 20(10); pp. 2763-2771;(2005).
- Huo et al.; "Corrosion of AZ91D Magnesium Alloy with a Chemical Conversion Coating and Electroless Nickel Layer"; Corrosion Science: 46; pp. 1467-1477; (2004).
- International Search Report and Written Opinion; International Application No. PCT/US2011/058099; International Filing Date: Oct. 27, 2011; Date of Mailing: May 11, 2012; 12 pages.
- Li, "Design of Abrasive Water Jet Perforation and Hydraulic Fracturing Tool," Oil Field Equipment, Mar. 2011.
- Li, et al., "Investigation of aluminium-based nanocomposites with ultra-high strength", Materials Science and Engineering A, 527, pp. 305-316, (2009).
- Liu, et al., "Calculated Phase Diagrams and the Corrosion of Die-Cast Mg-Al Alloys", Corrosion Science, 2009, 51, 606-619.
- International Search Report and Written Opinion, Date of Mailing Feb. 26, 2013; International Application No. PCT/US2012/047163, Korean Intellectual Property Office; Written Opinion 9 pages, International Search Report 3 pages.
- Baker Hughes Incorporated. IN-Tallic Disintegrating Frac Balls. Houston: Baker Hughes Incorporated, 2011. Accessed Mar. 6, 2015.
- Baker Hughes, "Multistage", Oct. 31, 2011, BakerHughes.com; accessed Mar. 6, 2015.
- International Search Report and Written Opinion; International Application No. PCT/US2012/071742; International Filing Date: Dec. 27, 2012; Date of Mailing: Apr. 22, 2013; 12 pages.
- International Search Report and Written Opinion; International Application No. PCT/US2014/058997, International Filing Date: Oct. 3, 2014; Date of Mailing: Jan. 12, 2015; 12 pages.
- International Search Report; International Application No. PCT/US2012/044229, International Filing Date: Jun. 26, 2012; Date of Mailing: Jan. 30, 2013; 3 pages.
- Murray, "Binary Alloy Phase Diagrams" Int. Met. Rev., 30(5) 1985 vol. 1, pp. 103-187.
- Vernon Constien et al., "Development of Reactive Coatings to Protect Sand-Control Screens", SPE 112494, Copyright 2008, Society of Petroleum Engineers, Presented at the 2008 SPE International Symposium and Exhibition on Formation Damage Control.



FIG. 1



FIG. 2



FIG. 3



FIG. 4



FIG. 5





FIG. 8



FIG. 9

## DEGRADABLE HIGH SHOCK IMPEDANCE MATERIAL

## CROSS REFERENCE TO RELATED APPLICATIONS

This application contains subject matter related to the subject matter of co-pending applications, which are assigned to the same assignee as this application, Baker Hughes Incorporated of Houston, Tex. and are all being filed on the same date as this application. The below listed applications are hereby incorporated by reference in their entirety:

U.S. patent application Ser. No. 13/225,414, filed Sep. 3, 2011, entitled "Degradable Shaped Charge and Perforating Gun System," and

U.S. patent application Ser. No. 13/225,415, filed Sep. 3, 2011, entitled "Method of Using a Degradable Shaped Charge and Perforating Gun System."

## BACKGROUND

To complete a well, one or more formation zones adjacent a wellbore are perforated to allow fluid from the formation zones to flow into the well for production to the surface or to allow injection fluids to be applied into the formation zones. Perforating systems are used for the purpose, among others, of making hydraulic communication passages, called perforations, in wellbores drilled through earth formations so that predetermined zones of the earth formations can be hydraulically connected to the wellbore. Perforations are needed because wellbores are typically completed by coaxially inserting a pipe or casing into the wellbore. The casing is retained in the wellbore by pumping cement into the annular space between the wellbore and the casing to line the wellbore. The cemented casing is provided in the wellbore for the specific purpose of hydraulically isolating from each other the various earth formations penetrated by the wellbore.

Perforating systems typically comprise one or more shaped charge perforating guns strung together. A perforating gun string may be lowered into the well and one or more guns fired to create openings in the casing and/or a cement liner and to extend perforations into the surrounding formation.

Shaped charge guns known in the art for perforating wellbores typically include a shaped charge liner. A high explosive is detonated to collapse the liner and ejects it from one end of the shaped charge at a very high velocity in a pattern called a "jet". The jet penetrates and perforates the casing, the cement and a quantity of the earth formation. In order to provide perforations which have efficient hydraulic communication with the formation, it is known in the art to design shaped charges in various ways to provide a jet which can penetrate a large quantity of formation, the quantity usually referred to as the "penetration depth" of the perforation. The jet from the metal liners also may leave a residue in the resulting perforation, thereby reducing the efficiency and productivity of the well.

Furthermore, once a shape charge gun has been fired, in addition to addressing the issues regarding the residual liner material left in the perforation, the components other than the liner must generally also be removed from the wellbore, which generally require additional costly and time consuming removal operations.

Therefore, perforation systems and methods of using them that incorporate liners and other components formed from materials that may be selectively removed from the wellbore are very desirable.

## SUMMARY

In an exemplary embodiment, a selectively corrodible powder compact is disclosed. The selectively corrodible powder compact includes a cellular nanomatrix comprising a nanomatrix material. The selectively corrodible powder compact also includes a plurality of dispersed particles comprising a particle core material having a density of about 7.5 g/cm<sup>3</sup> or more, dispersed in the cellular nanomatrix. The selectively corrodible powder compact further includes a bond layer extending throughout the cellular nanomatrix between the dispersed particles.

## BRIEF DESCRIPTION OF THE DRAWINGS

Referring now to the drawings wherein like elements are numbered alike in the several Figures:

FIG. 1 is a partial cutaway view of an exemplary embodiment of a perforating system and method of using the same as disclosed herein;

FIG. 2 is a cross-sectional view of an exemplary embodiment of a shaped charge as disclosed herein;

FIG. 3 is a perspective view of an exemplary embodiment of a perforating system, including shaped charges and a shaped charge housing as disclosed herein;

FIG. 4 is a cross-sectional view of an exemplary embodiment of a perforating system, including shaped charges, a shaped charge housing and an outer housing as disclosed herein;

FIG. 5 is a cross-sectional view of an exemplary embodiment of a coated powder as disclosed herein; and

FIG. 6 is a cross-sectional view of a nanomatrix material as may be used to make a selectively corrodible perforating system as disclosed herein;

FIG. 7 is a schematic of illustration of an exemplary embodiment of the powder compact have a substantially elongated configuration of dispersed particles as disclosed herein;

FIG. 8 is a schematic of illustration of an exemplary embodiment of the powder compact have a substantially elongated configuration of the cellular nanomatrix and dispersed particles, wherein the cellular nanomatrix and dispersed particles are substantially continuous; and

FIG. 9 is a schematic of illustration of an exemplary embodiment of the powder compact have a substantially elongated configuration of the cellular nanomatrix and dispersed particles, wherein the cellular nanomatrix and dispersed particles are substantially discontinuous.

## DETAILED DESCRIPTION

Generally, a selectively and controllably corrodible perforating system and method of using the perforating system for perforating a wellbore, either cased or open (i.e., uncased) is disclosed, as well as powder compact material compositions that may be used to form the various components of the selectively corrodible perforating system, particularly powder compacts comprising a cellular nanomatrix having a plurality particles of a particle core material dispersed therein. The selectively corrodible materials described herein may be corroded, dissolved or otherwise removed from the wellbore as described herein in response to a predetermined wellbore condition, such as exposure of the materials to a predetermined wellbore fluid, such as an acid, a fracturing fluid, an injection fluid, or a completions fluid, as described herein.

Referring to FIG. 1, after a well or wellbore 1 is drilled, a casing 70 is typically run in the wellbore 1 and cemented into

the well in order to maintain well integrity. After the casing 70 has been cemented with cement 72 in the wellbore 1, one or more sections of the casing 70 that are adjacent to the formation zones 3 of interest (e.g., target well zone) may be perforated to allow fluid from the formation zone 3 to flow into the well for production to the surface or to allow injection fluids to be applied into the formation zones 3. To perforate a casing 70 section, a selectively corrodible perforating system 4 comprising a selectively corrodible perforating gun 6 string may be lowered into the wellbore 1 to the desired depth of the formation zone 3 of interest, and one or more perforation guns 6 are fired to create openings 11 in the casing 70 and to extend perforations 10 into the formation zone 3. Production fluids in the perforated formation zone 3 can then flow through the perforations 10 and the casing openings 11 into the wellbore 1, for example.

Referring again to FIG. 1, an exemplary embodiment of a selectively corrodible perforating system 4 comprises one or more selectively corrodible perforating guns 6 strung together. These strings of guns 6 can have any suitable length, including a thousand feet or more of perforating length. For purposes of illustration, the perforating system 4 depicted comprises a single selectively corrodible perforating gun 6 rather than multiple guns. The gun 6 is shown disposed within a wellbore 1 on a wireline 5. As an example, the perforating system 4 as shown also includes a service truck 7 on the surface 9, where in addition to providing a raising and lowering system for the perforating system 4, the wireline 5 also may provide communication and control system between the truck 7 and the surface generally and the perforating gun 6 in the wellbore 1. The wireline 5 may be threaded through various pulleys and supported above the wellbore 1.

Perforating guns 6 includes a gun strip or shaped charge housing 16 that is configured to house one or more shaped charges 8 and that is coaxially housed within a gun body or outer housing 14. Both shaped charge housing 16 outer housing 14 may have any suitable shape, including an annular shape, and may be formed from any suitable material, including conventional housing materials, and in an exemplary embodiment either or both may be formed from a selectively corrodible material as described herein.

In an exemplary embodiment, shaped charge housing 16 may be formed from a selectively corrodible shaped charge housing material 17 as described herein. In another exemplary embodiment, outer housing 14 may be formed from a selectively corrodible material 15. The selectively corrodible outer housing material 15 and shaped charge housing material 17 may be the same material or different materials as described herein.

Shaped charges 8 are housed within the shaped charge housing 16 and aimed outwardly generally perpendicular to the axis of the wellbore 1. As illustrated in FIG. 2, in an exemplary embodiment a selectively corrodible shaped charge 8 includes a housing or charge case 18 formed from a selectively corrodible charge case material 19, a selectively corrodible shaped charge liner 22 formed from a selectively corrodible liner material 23 disposed within the charge case 18 generally axially along a longitudinal axis of the case, a quantity comprising a main charge 24 of high explosive material disposed within the charge case and deposited between the liner 22 and the charge case 18, and a booster charge 26 proximate the base of the high explosive 24 and configured for detonation of the high explosive.

Referring to FIG. 2, a shaped charge 8 in accordance with embodiments of the present invention includes a charge case 18 that acts as a containment vessel designed to hold the detonation force of the detonating explosion long enough for

a perforating jet 12 (FIGS. 1 and 2) to form. The case body 34 is a container-like structure having a bottom wall 33 section sloping upward with respect to the axis A of the charge case 18. The charge case 18 as shown is substantially symmetric about the axis A. In the embodiment shown, the charge case 18 transitions into the upper wall 35 portion where the slope of the wall steepens, including the orientation shown where the upper wall 35 is substantially parallel to the axis A. The upper portion 35 also has a profile oblique to the axis A. Extending downward from the bottom portion 33 is a cord slot 36 having a pair of tabs 25. The tabs 25 are configured to receive a detonating cord 27 therebetween and are generally parallel with the axis A of the charge case 18. A crown wall 41 portion defines the uppermost portion of the case body 34 extending from the upper terminal end of the upper portion 35. The uppermost portion of the crown portion 41 defines the opening 39 of the charge case 18 and lies in a plane that is substantially perpendicular to the axis A. A boss element 20 is provided on the outer surface of the crown portion 41. The boss 20 is an elongated member whose elongate section partially circumscribes a portion of the outer peripheral radius of the crown portion 41, and thus partially circumscribes the outer circumference of the charge case 18. In the embodiment shown, the boss 20 cross-section is substantially rectangular and extends radially outwardly from the outer surface of the charge case 18. While the charge case 8 shown is generally cylindrical, charge case 18 may have any shape suitable for housing the liner 22 and main charge 24 as described herein.

The shaped charges 8 may be positioned within the shaped charge housing 16 in any orientation or configuration, including a high density configuration of at least 10-12 shaped charges 8 per linear foot of perforating gun. In some instances however high density shots may include guns having as few as 6 shaped charge 8 shots per linear foot. Referring to FIG. 3, the shaped charge housing 16 provides an example of a high density configuration. The charges carried in a perforating gun 6 may be phased to fire in multiple directions around the circumference of the wellbore 1. Alternatively, the charges may be aligned in a straight line or in any predetermined firing pattern. When fired, the charges create perforating jets 12 that form openings 11 or perforations or holes in the surrounding casing 70 as well as extend perforations 10 into the surrounding formation zone 3.

FIG. 4 provides a view looking along the axis of the shaped charge housing 16 having multiple charge casings 18 disposed therein. In this view, a detonating cord 27 is shown coupled within the tabs 25 and cord slot 36 of the respective charge casings 18. The respective cord slots 36 of the charge cases 18 are aligned for receiving the detonation cord 27 therethrough. The shaped charge housing 16 is disposed within outer housing 14. As indicated the portion of outer housing 14 proximate shaped charges 8 may have the wall thickness reduced in a window, such as a generally circular window, either from the outer surface or inner surface, or both, to reduce the energy needed for the liner material to pierce through the housing and increase the energy available to penetrate the formation.

The liner 22 may have any suitable shape. In the exemplary embodiment of FIG. 2, the liner 22 is generally frustoconical in shape and is distributed substantially symmetrically about the axis A. Liner 22 generally may be described as having a sidewall 37 that defines an apex 21 and a liner opening 39. Other liner 22 shapes are also possible, including a multi-sectional liner having two or more frustoconical sections with different taper angles, such as one that opens at a first taper angle and a second taper angle that opens more rapidly than the first taper angle, a tulip-shaped liner, which as its name

suggest mimics the shape of a tulip, a fully or partially (e.g., combination of a cylindrical or frustoconical sidewall and hemispherical apex) hemispherical liner, a generally frustoconical liner having a rounded or curved apex, a linear liner having a V-shaped cross section with straight wall sides or a trumpet-shaped liner having generally conically shaped with curved sidewall that curve outwardly as they extend from the apex of the liner to the liner opening. Liner 22 may be formed as described herein to provide a porous powder compact having less than full theoretical density, so that the liner 22 substantially disintegrates into a perforating jet of particles upon detonation of the main charge 24 and avoids the formation of a "carrot" or "slug" of solid material. Liner 22 may also be formed as a solid material having substantially full theoretical density and the jet 12 formed therefrom may include a carrot 13 or slug. In either case, liner 22 is formed from selectively corrodible liner material 23 and is configured for removal of residual liner material 23 from the perforations 10 as described herein.

The main charge 24 is contained inside the charge case 18 and is arranged between the inner surface 31 of the charge case and the liner 22. A booster charge 26 or primer column or other ballistic transfer element is configured for explosively coupling the main explosive charge 24 and a detonating cord 27, which is attached to an end of the shaped charge, by providing a detonating link between them. Any suitable explosives may be used for the high explosive 24, booster charge 26 and detonating cord 27. Examples of explosives that may be used in the various explosive components (e.g., charges, detonating cord, and boosters) include RDX (cyclo-trimethylenetrinitramine or hexahydro-1,3,5-trinitro-1,3,5-triazine), HMX (cyclotetramethylenetrinitramine or 1,3,5,7-tetranitro-1,3,5,7-tetraazacyclooctane), TATB (triaminotrinitrobenzene), HNS (hexanitrostilbene), and others.

In an exemplary embodiment, in order to detonate the main charge 24 of shaped charge 8, a detonation wave traveling through the detonating cord 27 initiates the booster charge 26 when the detonation wave passes by, which in turn initiates detonation of the main explosive charge 24 to create a detonation wave that sweeps through the shaped charge. The liner 22 collapses under the detonation force of the main explosive charge. The shaped charges 8 are typically explosively coupled to or connected to a detonating cord 27 which is affixed to the shaped charge 8 by a case slot 25 and located proximate the booster charge 26. Detonating the detonating cord 27 creates a compressive pressure wave along its length that in turn detonates the booster charge 26 that in turn detonates the high explosive 24. When the high explosive 24 is detonated, the force of the detonation collapses the liner 22, generally pushing the apex 21 through the liner opening 39 and ejects it from one end of the shaped charge 8 at very high velocity in a pattern of the liner material that is called a perforating jet 12. The perforating jet 12 may have any suitable shape, but generally includes a high velocity pattern of fragments of the liner material on a leading edge and, particularly in the case of solid liner material 23, may also include a trailing carrot or slug comprising a substantially solid mass of the liner material. The perforating jet 12 is configured to shoot out of the open end 39 of the charge case 18 and perforate the outer housing 14, casing 70 and any cement 72 lining the wellbore 1 and create a perforation 10 in the formation 2, usually having the shape of a substantially conical or bullet-shaped funnel that tapers inwardly away from the wellbore 1 and extends into the surrounding earth formation 2. Around the surface region adjacent to the perforation 10 or tunnel, a layer of charge liner residue 50. The charge liner residue 50

includes "wall" residue 52 deposited on the wall of the perforation 10 and "tip" residue 54 deposited at the tip of the perforation. The selectively corrodible liner material 23 disclosed herein enables selective and rapid removal of the charge liner residue 50, including the wall residue 52 and tip residue 54 from the perforation in response to a predetermined wellbore condition, such as exposure of the charge liner residue 50 to a predetermined wellbore fluid of the types described herein. The removal of the charge liner residue, particularly the tip residue, is very advantageous, because it enables the unhindered flow of wellbore fluids into and out of the perforation through the tip portion, thereby increasing the productivity of the individual perforations and hence the overall productivity of the wellbore 1.

In accordance with embodiments of the present invention, the shaped charge 8 includes a liner 22 fabricated from a material that is selectively corrodible in the presence of a suitable predetermined wellbore fluid (e.g., an acid, an injection fluid, a fracturing fluid, or a completions fluid). As a result, any liner residue remaining in the perforation tunnel post-detonation (specifically, in the tip region of the tunnel) may be dissolved into the dissolving fluid and will no longer be detrimental to injection or other operations. It is significant that the material used in the charge liner be targeted to correspond with a dissolving fluid in which the liner material is soluble in presence of Perforating system 4 may also include a galvanic member 60, such as a metallic or conductive member, that is selected to promote galvanic coupling and dissolution or corrosion of the selectively corrodible members, particularly one or more of charge cases 18, shape charge housing 16 or outer housing 14.

Once the shaped charges 8 have been fired, it is also desirable to remove remaining portions of the perforating system 4 from the wellbore, particularly the shaped charge case 18, shaped charge housing 16 and outer housing 14. In an exemplary embodiment, where charge case 18 is formed from selectively corrodible charge case material 19, and one or both of shaped charge housing 16 and outer housing 14 is formed from selectively corrodible shaped charge housing material 17 and selectively corrodible outer housing material 15, respectively, the remaining portions of perforating system 4 that are formed from a selectively corrodible material may be removed from the wellbore by exposure to a predetermined wellbore fluid, as described herein. The remainder of the perforating system 4 may be selectively corroded, dissolved or otherwise removed from the wellbore at the same time as the charge liner residue 50 by exposure to the same predetermined wellbore fluid. Alternately, the remainder of perforating system 4 may be removed from the wellbore at a different time by exposure to a different predetermined wellbore fluid.

As described, the selectively corrodible materials described herein may be corroded, dissolved or otherwise removed from the wellbore as described herein in response to a predetermined wellbore condition, such as exposure of the materials to a predetermined wellbore fluid, such as an acid, a fracturing fluid, an injection fluid, or a completions fluid, as described herein. Acids that may be used to dissolve any charge liner residue in acidizing operations include, but are not limited to: hydrochloric acid, hydrofluoric acid, acetic acid, and formic acid. Fracturing fluids that may be used to dissolve any charge liner residue in fracturing operations include, but are not limited to: acids, such as hydrochloric acid and hydrofluoric acid. Injection fluids that may be pumped into the formation interval to dissolve any charge liner residue include, but are not limited to: water and seawater. Completion fluids that may be circulated proximate the

formation interval to dissolve any charge liner residue include, but are not limited to, brines, such as chlorides, bromides and formates.

A method for perforating in a well include: (1) disposing a perforating gun in the well, wherein the perforating gun comprises a shaped charge having a charge case, an explosive disposed inside the charge case, and a liner for retaining the explosive in the charge case, wherein the liner includes a material that is soluble with an acid, an injection fluid, a fracturing fluid, or a completions fluid; (2) detonating the shaped charge to form a perforation tunnel in a formation zone and leaving charge liner residue within the perforating tunnel (on the well and tip); (3) performing one of the following: (i) pumping an acid downhole, (ii) pumping a fracturing fluid downhole, (iii) pumping an injection fluid downhole, or (iv) circulating a completion or wellbore fluid downhole to contact the charge liner residue in the perforation tunnel; and (4) allowing the material comprising the charge liner residue to dissolve with the acid, an injection fluid, a fracturing fluid, or a completions fluid. After such operation, a treatment fluid may be injected into the formation and/or the formation may be produced.

In an exemplary embodiment, the selectively corrodible perforating system **4** components described herein may be formed from selectively corrodible nanomatrix materials. These include: the shaped charge **8** comprising shaped charge housing **16** and shaped charge housing material **19** and liner **22** and selectively corrodible liner material **23**, shaped charge housing **16** and selectively corrodible shaped charge housing material **17**, and outer housing **14** and selectively corrodible outer housing material **15**. The Nanomatrix materials and methods of making these materials are described generally, for example, in U.S. patent application Ser. No. 12/633,682 filed on Dec. 8, 2009 and U.S. patent application Ser. No. 13/194,361 filed on Jul. 29, 2011, which are hereby incorporated herein by reference in their entirety. These lightweight, high-strength and selectively and controllably degradable materials may range from fully-dense, sintered powder compacts to precursor or green state (less than fully dense) compacts that may be sintered or unsintered. They are formed from coated powder materials that include various lightweight particle cores and core materials having various single layer and multilayer nanoscale coatings. These powder compacts are made from coated metallic powders that include various electrochemically-active (e.g., having relatively higher standard oxidation potentials) lightweight, high-strength particle cores and core materials, such as electrochemically active metals, that are dispersed within a cellular nanomatrix formed from the consolidation of the various nanoscale metallic coating layers of metallic coating materials, and are particularly useful in wellbore applications. The powder compacts may be made by any suitable powder compaction method, including cold isostatic pressing (CIP), hot isostatic pressing (HIP), dynamic forging and extrusion, and combinations thereof. These powder compacts provide a unique and advantageous combination of mechanical strength properties, such as compression and shear strength, low density and selectable and controllable corrosion properties, particularly rapid and controlled dissolution in various wellbore fluids. The fluids may include any number of ionic fluids or highly polar fluids, such as those that contain various chlorides. Examples include fluids comprising potassium chloride (KCl), hydrochloric acid (HCl), calcium chloride (CaCl<sub>2</sub>), calcium bromide (CaBr<sub>2</sub>) or zinc bromide (ZnBr<sub>2</sub>). The disclosure of the '682 and '361 applications regarding the nature of the coated powders and methods of making and compacting the coated powders are generally applicable to

provide the selectively corrodible nanomatrix materials disclosed herein, and for brevity, are not repeated herein.

As illustrated in FIGS. 1 and 2, the selectively corrodible materials disclosed herein may be formed from a powder **100** comprising powder particles **112**, including a particle core **114** and core material **118** and metallic coating layer **116** and coating material **120**, may be selected that is configured for compaction and sintering to provide a powder metal compact **200** that is selectively and controllably removable from a wellbore in response to a change in a wellbore property, including being selectively and controllably dissolvable in a predetermined wellbore fluid, including various predetermined wellbore fluids as disclosed herein. The powder metal compact **200** includes a cellular nanomatrix **216** comprising a nanomatrix material **220** and a plurality of dispersed particles **214** comprising a particle core material **218** as described herein dispersed in the cellular nanomatrix **216**.

As described herein, the shaped charge **8** comprising shaped charge housing **16** and shaped charge housing material **19** and liner **22** and selectively corrodible liner material **23**, shaped charge housing **16** and selectively corrodible shaped charge housing material **17**, and outer housing **14** and selectively corrodible outer housing material **15** may be formed from the same materials or different materials. In an exemplary embodiment, it is desirable to form the shaped charge **8**, including the shaped charge housing **16** or liner **22**, or both of them, from a nanomatrix material that provides a mechanical shock impedance or mechanical shock response that enables containment of the explosion by the shaped charge housing **16** and formation of jet **12** from liner **22** that is configured to penetrate various earth formations, such as, for example, materials having a high density and ductility. In another exemplary embodiment, it is desirable to form the shaped charge housing **16** or outer housing **14**, or both of them, from a lightweight, high-strength material sufficient to house the shaped charges **8**.

Dispersed particles **214** may comprise any of the materials described herein for particle cores **114**, even though the chemical composition of dispersed particles **214** may be different due to diffusion effects as described herein. In an exemplary embodiment, the shaped charge **8**, including the shaped charge housing **16** and liner **22**, may include dispersed particles **214** that are formed from particle cores **114** with particle core material having a density of about 7.5 g/cm<sup>3</sup> or more, and more particularly a density of about 8.5 g/cm<sup>3</sup> or more, and even more particularly a density of about 10 g/cm<sup>3</sup> or more. More particularly, particle cores **114** may include a particle core material **118** that comprises a metal, ceramic, cermet, glass or carbon, or a composite thereof, or a combination of any of the foregoing materials. Even more particularly, particle cores **114** may include a particle core material **118** that comprises Fe, Ni, Cu, W, Mo, Ta, U or Co, or a carbide, oxide or nitride comprising at least one of the foregoing metals, or an alloy comprising at least one of the aforementioned materials, or a composite comprising at least one of the aforementioned materials, or a combination of any of the foregoing. If uranium is used, it may include depleted uranium, since it is commercially more readily available. The dispersed particles **214** may be formed from a single particle core material or multiple particle core materials. In one embodiment, dispersed particles **214** are formed from particle cores **114** that comprise up to about 50 volume percent of an Mg—Al alloy, such as an alloy of Mg-10 wt. % Al, and about 50 volume percent or more of a W—Al alloy, such as an alloy of W-10 wt. % Al. In another embodiment, dispersed particles **214** are formed from particle cores **114** that comprise up to about 50 volume percent of an Mg—Al alloy, such

as an alloy of Mg-10 wt. % Al, and about 50 volume percent or more of a Zn—Al alloy, such as an alloy of Zn-10 wt. % Al. In yet another embodiment, dispersed particles **214** are formed from particle cores **114** that comprise up to about 50 volume percent of an Mg—Ni alloy, such as an alloy of Mg-5 wt. % Ni, and about 50 volume percent or more of a W—Ni alloy, such as an alloy of W-5 wt. % Ni. In these embodiments that are formed from a mixture of different powders **110** and powder particles **112** having different particle core materials **118**, at least a portion (e.g., 50 volume percent or more) of the particle cores **114** have a density greater than 7.5 g/cm<sup>3</sup>. In other embodiments, dispersed particles **214** may be formed from a powder **100** having powder particles **112** with particle cores **114** formed from particle core materials **118** that include alloys, wherein the alloy has a density greater than about 7.5 g/cm<sup>3</sup>, such as may be formed from binary, ternary, etc. alloys having at least one alloy constituent with a density greater than about 7.5 g/cm<sup>3</sup>. The particle cores **114** and particle core material of the liner **22** are preferably formed from ductile materials. In an exemplary embodiment, ductile materials include materials that exhibit 5% or more of true strain or elongation at failure or breaking.

In an exemplary embodiment, the shaped charge housing **16** and/or outer housing **14** may include dispersed particles **214** that are formed from particle cores **114** with any suitable particle core material, including, in one embodiment, the same particle core materials used to form the components of shaped charge **8**. In another exemplary embodiment, they may be formed from dispersed particles **214** that are formed from particle cores **114** having a particle core material **118** comprising Mg, Al, Zn or Mn, or alloys thereof, or a combination thereof.

Dispersed particles **214** and particle core material **218** may also include a rare earth element, or a combination of rare earth elements. As used herein, rare earth elements include Sc, Y, La, Ce, Pr, Nd or Er, or a combination of rare earth elements. Where present, a rare earth element or combination of rare earth elements may be present, by weight, in an amount of about 5 percent or less.

Powder compact **200** includes a cellular nanomatrix **216** of a nanomatrix material **220** having a plurality of dispersed particles **214** dispersed throughout the cellular nanomatrix **216**. The dispersed particles **214** may be equiaxed in a substantially continuous cellular nanomatrix **216**, or may be substantially elongated as described herein and illustrated in FIG. 3. In the case where the dispersed particles **214** are substantially elongated, the dispersed particles **214** and the cellular nanomatrix **216** may be continuous or discontinuous, as illustrated in FIGS. 4 and 5, respectively. The substantially continuous cellular nanomatrix **216** and nanomatrix material **220** formed of sintered metallic coating layers **116** is formed by the compaction and sintering of the plurality of metallic coating layers **116** of the plurality of powder particles **112**, such as by CIP, HIP or dynamic forging. The chemical composition of nanomatrix material **220** may be different than that of coating material **120** due to diffusion effects associated with the sintering. Powder metal compact **200** also includes a plurality of dispersed particles **214** that comprise particle core material **218**. Dispersed particle **214** and core material **218** correspond to and are formed from the plurality of particle cores **114** and core material **118** of the plurality of powder particles **112** as the metallic coating layers **116** are sintered together to form nanomatrix **216**. The chemical composition of core material **218** may also be different than that of core material **118** due to diffusion effects associated with sintering.

As used herein, the use of the term cellular nanomatrix **216** does not connote the major constituent of the powder compact, but rather refers to the minority constituent or constituents, whether by weight or by volume. This is distinguished from most matrix composite materials where the matrix comprises the majority constituent by weight or volume. The use of the term substantially-continuous, cellular nanomatrix is intended to describe the extensive, regular, continuous and interconnected nature of the distribution of nanomatrix material **220** within powder compact **200**. As used herein, “substantially-continuous” describes the extension of the nanomatrix material throughout powder compact **200** such that it extends between and envelopes substantially all of the dispersed particles **214**. Substantially-continuous is used to indicate that complete continuity and regular order of the nanomatrix around each dispersed particle **214** is not required. For example, defects in the coating layer **116** over particle core **114** on some powder particles **112** may cause bridging of the particle cores **114** during sintering of the powder compact **200**, thereby causing localized discontinuities to result within the cellular nanomatrix **216**, even though in the other portions of the powder compact the nanomatrix is substantially continuous and exhibits the structure described herein. In contrast, in the case of substantially elongated dispersed particles **214**, such as those formed by extrusion, “substantially discontinuous” is used to indicate that incomplete continuity and disruption (e.g., cracking or separation) of the nanomatrix around each dispersed particle **214**, such as may occur in a predetermined extrusion direction **622**, or a direction transverse to this direction. As used herein, “cellular” is used to indicate that the nanomatrix defines a network of generally repeating, interconnected, compartments or cells of nanomatrix material **220** that encompass and also interconnect the dispersed particles **214**. As used herein, “nanomatrix” is used to describe the size or scale of the matrix, particularly the thickness of the matrix between adjacent dispersed particles **214**. The metallic coating layers that are sintered together to form the nanomatrix are themselves nanoscale thickness coating layers. Since the nanomatrix at most locations, other than the intersection of more than two dispersed particles **214**, generally comprises the interdiffusion and bonding of two coating layers **16** from adjacent powder particles **112** having nanoscale thicknesses, the matrix formed also has a nanoscale thickness (e.g., approximately two times the coating layer thickness as described herein) and is thus described as a nanomatrix. Further, the use of the term dispersed particles **214** does not connote the minor constituent of powder compact **200**, but rather refers to the majority constituent or constituents, whether by weight or by volume. The use of the term dispersed particle is intended to convey the discontinuous and discrete distribution of particle core material **218** within powder compact **200**.

Particle cores **114** and dispersed particles **214** of powder compact **200** may have any suitable particle size. In an exemplary embodiment, the particle cores **114** may have a unimodal distribution and an average particle diameter or size of about 5 µm to about 300 µm, more particularly about 80 µm to about 120 µm, and even more particularly about 100 µm. In another exemplary embodiment, which may include a multimodal distribution of particle sizes, the particle cores **114** may have average particle diameters or size of about 50 nm to about 500 µm, more particularly about 500 nm to about 300 µm, and even more particularly about 5 µm to about 300 µm. In an exemplary embodiment, the particle cores **114** or the dispersed particles may have an average particle size of about 50 nm to about 500 µm.

## 11

Dispersed particles 214 may have any suitable shape depending on the shape selected for particle cores 114 and powder particles 112, as well as the method used to sinter and compact powder 100. In an exemplary embodiment, powder particles 112 may be spheroidal or substantially spheroidal and dispersed particles 214 may include an equiaxed particle configuration as described herein. In another exemplary embodiment as shown in FIGS. 7-9, dispersed particles may have a non-spherical shape. In yet another embodiment, the dispersed particles may be substantially elongated in a predetermined extrusion direction 622, such as may occur when using extrusion to form powder compact 200. As illustrated in FIG. 3-5, for example, a substantially elongated cellular nanomatrix 616 comprising a network of interconnected elongated cells of nanomatrix material 620 having a plurality of substantially elongated dispersed particle cores 614 of core material 618 disposed within the cells. Depending on the amount of deformation imparted to form elongated particles, the elongated coating layers and the nanomatrix 616 may be substantially continuous in the predetermined direction 622 as shown in FIG. 4, or substantially discontinuous as shown in FIG. 5.

The nature of the dispersion of dispersed particles 214 may be affected by the selection of the powder 100 or powders 100 used to make particle compact 200. In one exemplary embodiment, a powder 100 having a unimodal distribution of powder particle 112 sizes may be selected to form powder compact 200 and will produce a substantially homogeneous unimodal dispersion of particle sizes of dispersed particles 214 within cellular nanomatrix 216. In another exemplary embodiment, a plurality of powders 100 having a plurality of powder particles with particle cores 114 that have the same core materials 118 and different core sizes and the same coating material 120 may be selected and uniformly mixed as described herein to provide a powder 100 having a homogeneous, multimodal distribution of powder particle 112 sizes, and may be used to form powder compact 200 having a homogeneous, multimodal dispersion of particle sizes of dispersed particles 214 within cellular nanomatrix 216. Similarly, in yet another exemplary embodiment, a plurality of powders 10 having a plurality of particle cores 114 that may have the same core materials 118 and different core sizes and the same coating material 120 may be selected and distributed in a non-uniform manner to provide a non-homogeneous, multimodal distribution of powder particle sizes, and may be used to form powder compact 200 having a non-homogeneous, multimodal dispersion of particle sizes of dispersed particles 214 within cellular nanomatrix 216. The selection of the distribution of particle core size may be used to determine, for example, the particle size and interparticle spacing of the dispersed particles 214 within the cellular nanomatrix 216 of powder compacts 200 made from powder 100.

As illustrated generally in FIGS. 5 and 6, powder metal compact 200 may also be formed using coated metallic powder 100 and an additional or second powder 130, as described herein. The use of an additional powder 130 provides a powder compact 200 that also includes a plurality of dispersed second particles 234, as described herein, that are dispersed within the nanomatrix 216 and are also dispersed with respect to the dispersed particles 214. Dispersed second particles 234 may be formed from coated or uncoated second powder particles 132, as described herein. In an exemplary embodiment, coated second powder particles 132 may be coated with a coating layer 136 that is the same as coating layer 116 of powder particles 112, such that coating layers 136 also contribute to the nanomatrix 216. In another exemplary embodiment, the second powder particles 234 may be uncoated such

## 12

that dispersed second particles 234 are embedded within nanomatrix 216. As disclosed herein, powder 100 and additional powder 130 may be mixed to form a homogeneous dispersion of dispersed particles 214 and dispersed second particles 234 or to form a non-homogeneous dispersion of these particles. The dispersed second particles 234 may be formed from any suitable additional powder 130 that is different from powder 100, either due to a compositional difference in the particle core 134, or coating layer 136, or both of them, and may include any of the materials disclosed herein for use as second powder 130 that are different from the powder 100 that is selected to form powder compact 200. In an exemplary embodiment, dispersed second particles 234 may include Ni, Fe, Cu, Co, W, Al, Zn, Mn or Si, or an oxide, nitride, carbide, intermetallic compound or cermet comprising at least one of the foregoing, or a combination thereof.

Nanomatrix 216 is formed by sintering metallic coating layers 116 of adjacent particles to one another by interdiffusion and creation of bond layer 219 as described herein. Metallic coating layers 116 may be single layer or multilayer structures, and they may be selected to promote or inhibit diffusion, or both, within the layer or between the layers of metallic coating layer 116, or between the metallic coating layer 116 and particle core 114, or between the metallic coating layer 116 and the metallic coating layer 116 of an adjacent powder particle, the extent of interdiffusion of metallic coating layers 116 during sintering may be limited or extensive depending on the coating thicknesses, coating material or materials selected, the sintering conditions and other factors. Given the potential complexity of the interdiffusion and interaction of the constituents, description of the resulting chemical composition of nanomatrix 216 and nanomatrix material 220 may be simply understood to be a combination of the constituents of coating layers 16 that may also include one or more constituents of dispersed particles 214, depending on the extent of interdiffusion, if any, that occurs between the dispersed particles 214 and the nanomatrix 216. Similarly, the chemical composition of dispersed particles 214 and particle core material 218 may be simply understood to be a combination of the constituents of particle core 114 that may also include one or more constituents of nanomatrix 216 and nanomatrix material 220, depending on the extent of interdiffusion, if any, that occurs between the dispersed particles 214 and the nanomatrix 216.

In an exemplary embodiment, the nanomatrix material 220 has a chemical composition and the particle core material 218 has a chemical composition that is different from that of nanomatrix material 220, and the differences in the chemical compositions may be configured to provide a selectable and controllable dissolution rate, including a selectable transition from a very low dissolution rate to a very rapid dissolution rate, in response to a controlled change in a property or condition of the wellbore proximate the compact 200, including a property change in a wellbore fluid that is in contact with the powder compact 200, as described herein. Nanomatrix 216 may be formed from powder particles 112 having single layer and multilayer coating layers 116. This design flexibility provides a large number of material combinations, particularly in the case of multilayer coating layers 116, that can be utilized to tailor the cellular nanomatrix 216 and composition of nanomatrix material 220 by controlling the interaction of the coating layer constituents, both within a given layer, as well as between a coating layer 116 and the particle core 114 with which it is associated or a coating layer 116 of an adjacent powder particle 112. Several exemplary embodiments that demonstrate this flexibility are provided below.

As illustrated in FIGS. 5 and 6, in an exemplary embodiment, powder compact 200 is formed from powder particles 112 where the coating layer 116 comprises a single layer, and the resulting nanomatrix 216 between adjacent ones of the plurality of dispersed particles 214 comprises the single metallic coating layer 116 of one powder particle 112, a bond layer 219 and the single coating layer 116 of another one of the adjacent powder particles 112. The thickness of bond layer 219 is determined by the extent of the interdiffusion between the single metallic coating layers 116, and may encompass the entire thickness of nanomatrix 216 or only a portion thereof. In other words, the compact is formed from a sintered powder 100 comprising a plurality of powder particles 112, each powder particle 112 having a particle core that upon sintering comprises a dispersed particle 214 and a single metallic coating layer 116 disposed thereon, and wherein the cellular nanomatrix 216 between adjacent ones of the plurality of dispersed particles 214 comprises the single metallic coating layer 116 of one powder particle 116, the bond layer 219 and the single metallic coating layer 116 of another of the adjacent powder particles 112. In another embodiment, the powder compact 200 is formed from a sintered powder 100 comprising a plurality of powder particles 112, each powder particle 112 having a particle core 114 that upon sintering comprises a dispersed particle 214 and a plurality of metallic coating layers 116 disposed thereon, and wherein the cellular nanomatrix 216 between adjacent ones of the plurality of dispersed particles 214 comprises the plurality of metallic coating layers 116 of one powder particle 112, the bond layer 219 and the plurality of metallic coating layers 116 of another of the powder particles 112, and wherein adjacent ones of the plurality of metallic coating layers 116 have different chemical compositions.

The cellular nanomatrix 216 may have any suitable nanoscale thickness. In an exemplary embodiment, the cellular nanomatrix 216 has an average thickness of about 50 nm to about 5000 nm.

In one exemplary embodiment, nanomatrix 216 may include Al, Zn, Mn, Mg, Mo, W, Cu, Fe, Si, Ca, Co, Ta, Re or Ni, or an oxide, carbide or nitride thereof, or a combination of any of the aforementioned materials, including combinations where the nanomatrix material 220 of cellular nanomatrix 216, including bond layer 219, has a chemical composition and the core material 218 of dispersed particles 214 has a chemical composition that is different than the chemical composition of nanomatrix material 220. The difference in the chemical composition of the nanomatrix material 220 and the core material 218 may be used to provide selectable and controllable dissolution in response to a change in a property of a wellbore, including a wellbore fluid, as described herein.

Powder compact 200 may have any desired shape or size, including that of a cylindrical billet, bar, sheet or other form that may be machined, formed or otherwise used to form useful articles of manufacture, including various wellbore tools and components. The pressing used to form precursor powder compact 100 and sintering and pressing processes used to form powder compact 200 and deform the powder particles 112, including particle cores 114 and coating layers 116, to provide the full density and desired macroscopic shape and size of powder compact 200 as well as its microstructure. The morphology (e.g., equiaxed or substantially elongated) of the dispersed particles 214 and nanomatrix 216 of particle layers results from sintering and deformation of the powder particles 112 as they are compacted and interdif-

fuse and deform to fill the interparticle spaces 115 (FIG. 1). The sintering temperatures and pressures may be selected to ensure that the density of powder compact 200 achieves substantially full theoretical density.

The powder compact 200 may be formed by any suitable forming method, including uniaxial pressing, isostatic pressing, roll forming, forging, or extrusion at a forming temperature. The forming temperature may be any suitable forming temperature. In one embodiment, the forming temperature may comprise an ambient temperature, and the powder compact 200 may have a density that is less than the full theoretical density of the particles 112 that form compact 200, and may include porosity. In another embodiment, the forming temperature the forming temperature may comprise a temperature that is about is about 20° C. to about 300° C. below a melting temperature of the powder particles, and the powder compact 200 may have a density that is substantially equal to the full theoretical density of the particles 112 that form the compact, and may include substantially no porosity.

The terms “a” and “an” herein do not denote a limitation of quantity, but rather denote the presence of at least one of the referenced items. The modifier “about” used in connection with a quantity is inclusive of the stated value and has the meaning dictated by the context (e.g., includes the degree of error associated with measurement of the particular quantity). Furthermore, unless otherwise limited all ranges disclosed herein are inclusive and combinable (e.g., ranges of “up to about 25 weight percent (wt. %), more particularly about 5 wt. % to about 20 wt. % and even more particularly about 10 wt. % to about 15 wt. %” are inclusive of the endpoints and all intermediate values of the ranges, e.g., “about 5 wt. % to about 25 wt. %, about 5 wt. % to about 15 wt. %”, etc.). The use of “about” in conjunction with a listing of constituents of an alloy composition is applied to all of the listed constituents, and in conjunction with a range to both endpoints of the range. Finally, unless defined otherwise, technical and scientific terms used herein have the same meaning as is commonly understood by one of skill in the art to which this invention belongs. The suffix “(s)” as used herein is intended to include both the singular and the plural of the term that it modifies, thereby including one or more of that term (e.g., the metal(s) includes one or more metals). Reference throughout the specification to “one embodiment”, “another embodiment”, “an embodiment”, and so forth, means that a particular element (e.g., feature, structure, and/or characteristic) described in connection with the embodiment is included in at least one embodiment described herein, and may or may not be present in other embodiments.

It is to be understood that the use of “comprising” in conjunction with the alloy compositions described herein specifically discloses and includes the embodiments wherein the alloy compositions “consist essentially of” the named components (i.e., contain the named components and no other components that significantly adversely affect the basic and novel features disclosed), and embodiments wherein the alloy compositions “consist of” the named components (i.e., contain only the named components except for contaminants which are naturally and inevitably present in each of the named components).

While one or more embodiments have been shown and described, modifications and substitutions may be made thereto without departing from the spirit and scope of the invention. Accordingly, it is to be understood that the present invention has been described by way of illustrations and not limitation.

## 15

The invention claimed is:

1. A selectively corrodible powder compact, comprising: a cellular nanomatrix comprising a nanomatrix material; a plurality of dispersed particles comprising a plurality of different particle core materials dispersed in the cellular nanomatrix, 50 volume percent or more of the particle core materials comprising a metal having a density of about 7.5 g/cm<sup>3</sup> or more; and a bond layer extending throughout the cellular nanomatrix between the dispersed particles.

2. The powder compact of claim 1, wherein the particle core materials further comprise at least one of ceramic, cermet, glass or carbon, or a composite thereof, or a combination of any of the foregoing materials.

3. The powder compact of claim 1, wherein the particle core materials comprise Fe, Ni, Cu, W, Mo, Ta, U or Co, or a carbide, oxide or nitride comprising at least one of the foregoing metals, or an alloy comprising at least one of the aforementioned materials, or a composite comprising at least one of the aforementioned materials, or a combination of any of the foregoing.

4. The powder compact of claim 1, wherein the particle core materials are ductile.

5. The powder compact of claim 1, wherein the dispersed particles further comprise a rare earth element.

6. The powder compact of claim 1, wherein the dispersed particles have an average particle size of about 50 nm to about 500  $\mu$ m.

7. The powder compact of claim 1, wherein the dispersion of dispersed particles comprises a substantially homogeneous dispersion within the cellular nanomatrix.

8. The powder compact of claim 1, wherein the dispersion of dispersed particles comprises a multi-modal distribution of dispersed particle sizes within the cellular nanomatrix.

9. The powder compact of claim 1, wherein the dispersed particles have an equiaxed particle shape or a substantially elongated particle shape.

10. The powder compact of claim 1, further comprising a plurality of dispersed second particles, the dispersed second particle having a density greater than 7.5 g/cm<sup>3</sup>, wherein the dispersed second particles are also dispersed within the cellular nanomatrix and with respect to the dispersed particles.

11. The powder compact of claim 10, wherein the dispersed second particles comprise Fe, Ni, Cu, or Co, or a carbide, oxide or nitride comprising at least one of the foregoing metals, or an alloy comprising at least one of the aforementioned materials, or a composite comprising at least one of the aforementioned materials, or a combination of any of the foregoing.

12. The powder compact of claim 1, wherein the nanomatrix material comprises Al, Zn, Mn, Mg, Mo, W, Cu, Fe, Si, Ca, Co, Ta, Re or Ni, or an oxide, carbide or nitride thereof, or a combination of any of the aforementioned materials, and wherein the nanomatrix material has a chemical composition and the particle core material has a chemical composition that is different than the chemical composition of the nanomatrix material.

## 16

13. The powder compact of claim 1, wherein the cellular nanomatrix has an average thickness of about 50 nm to about 5000 nm.

14. The powder compact of claim 1, wherein the compact is formed from a sintered powder comprising a plurality of powder particles, each powder particle having a particle core that upon sintering comprises a dispersed particle and a single metallic coating layer disposed thereon, and wherein the cellular nanomatrix between adjacent ones of the plurality of dispersed particles comprises the single metallic coating layer of one powder particle, the bond layer and the single metallic coating layer of another of the powder particles.

15. The powder metal compact of claim 1, wherein the compact is formed from a sintered powder comprising a plurality of powder particles, each powder particle having a particle core that upon sintering comprises a dispersed particle and a plurality of metallic coating layers disposed thereon, and wherein the cellular nanomatrix between adjacent ones of the plurality of dispersed particles comprises the plurality of metallic coating layers of one powder particle, the bond layer and plurality of metallic coating layers of another of the powder particles, and wherein adjacent ones of the plurality of metallic coating layers have different chemical compositions.

16. The powder compact of claim 1, wherein the powder compact comprises a plurality of unsintered powder particles.

17. The powder compact of claim 16, wherein the powder compact has a density that is less than a theoretical density of the powder particles.

18. The powder compact of claim 16, wherein the powder compact is formed by a method of uniaxial pressing, isostatic pressing, roll forming, forging, or extrusion at a forming temperature.

19. The powder compact of claim 18, wherein the forming temperature comprises an ambient temperature.

20. The powder compact of claim 1, wherein the powder compact comprises a plurality of sintered powder particles.

21. The powder compact of claim 20, wherein the powder compact has a density that is substantially the same as a theoretical density of the powder particles.

22. The powder compact of claim 20, wherein the powder compact is formed by a method of uniaxial pressing, isostatic pressing, roll forming, forging, or extrusion at a forming temperature.

23. The powder compact of claim 22, wherein the forming temperature is about 20° C. to about 300° C. below a melting temperature of the powder particles.

24. The powder compact of claim 1, wherein at least one of the particle core materials has a density of about 8.5 g/cm<sup>3</sup> or more.

25. The powder compact of claim 1, wherein at least one of the particle core materials has a density of about 10 g/cm<sup>3</sup> or more.

\* \* \* \* \*